



US006458525B1

(12) **United States Patent**  
Takiguchi et al.

(10) **Patent No.:** US 6,458,525 B1  
(45) **Date of Patent:** Oct. 1, 2002

(54) **PREPARATION METHOD OF PHOTOTHERMOGRAPHIC MATERIAL**

(75) Inventors: **Hideki Takiguchi; Hitoshi Adachi; Hideki Hoshino; Shu Nishiwaki**, all of Hino (JP)

(73) Assignee: **Konica Corporation (JP)**

(\*) Notice: Subject to any disclaimer, the term of this patent is extended or adjusted under 35 U.S.C. 154(b) by 0 days.

(21) Appl. No.: **09/705,592**

(22) Filed: **Nov. 3, 2000**

(30) **Foreign Application Priority Data**

Nov. 11, 1999 (JP) ..... 11-321162  
Dec. 7, 1999 (JP) ..... 11-347614

(51) **Int. Cl.<sup>7</sup>** ..... G03C 1/498; G03C 1/015;  
B65B 29/00

(52) **U.S. Cl.** ..... 430/617; 430/607; 430/619;  
430/927; 430/935; 206/455; 53/402; 53/432;  
53/510

(58) **Field of Search** ..... 430/617, 619,  
430/620, 607, 935, 927; 53/402, 432, 510;  
206/455

(56) **References Cited**

U.S. PATENT DOCUMENTS

4,273,723 A \* 6/1981 Hayashi et al. ..... 260/414  
4,305,844 A \* 12/1981 Vangermain et al. ..... 252/443  
5,382,504 A \* 1/1995 Shor et al. ..... 430/619  
5,637,550 A 6/1997 Leenders  
6,043,834 A \* 3/2000 Torisawa ..... 347/218  
6,083,681 A \* 7/2000 Lynch et al. ..... 430/619

OTHER PUBLICATIONS

European Search Report EP 00 30 9966.  
1 pg. of XP-002]84339, English Abstract only.

\* cited by examiner

*Primary Examiner*—Thorl Chea

(74) *Attorney, Agent, or Firm*—Bierman, Muserlian and Lucas

(57) **ABSTRACT**

A method for preparing a photothermographic material comprising an organic silver salt is disclosed, comprising a step of treating the organic silver salt under a gas atmosphere containing an inert gas having a volume fraction of not less than 85% or under a gas atmosphere containing oxygen gas having a volume fraction of not more than 15%. Packaging the photothermographic material under the inert gas atmosphere is also disclosed.

17 Claims, 1 Drawing Sheet



FIG. 1



**PREPARATION METHOD OF  
PHOTOTHERMOGRAPHIC MATERIAL**

**FIELD OF THE INVENTION**

The present invention relates to photothermographic materials exhibiting superior storage stability and in particular to black-and-white photothermographic materials exhibiting superior storage stability of silver images.

**BACKGROUND OF THE INVENTION**

In the field of medical treatment and graphic arts, there have been problems in working property with respect to effluents produced from wet-processing of image forming materials, and recently, reduction of the processing effluent 15 is strongly demanded in terms of environment protection and space saving.

Accordingly, there are needed techniques regarding photothermographic materials for photographic use and which are capable of forming black images exhibiting high 20 sharpness, enabling efficient exposure by means of a laser imager or laser image setter. As such a technique is known a photothermographic material, which comprises a support having thereon an organic silver salt, light-sensitive silver halide grains and a reducing agent, as described in U.S. Pat. No. 3,152,904 and 3,487,075; and D. Morgan "Dry Silver Photographic Material" (Handbook of Imaging Materials, Marcel Dekker, Inc., page 48, 1991). No processing solution is used in this photothermographic material (hereinafter, also referred to as a photothermographic material), enabling a 30 simple system friendly to the environment and operators.

Since this thermally developable photothermographic material contains an organic silver salt, light-sensitive silver halide grains and a reducing agent, there are problems such that the photothermographic material not only tends to cause fogging before or during thermal development but also 35 easily produces fog or photolytic silver (or print-out silver). Specifically, this photothermographic material, after exposure, is subjected only to thermal development at a temperature of 80 to 250° C., without being further subjected to fixing so that there were such problems that silver images causes discoloring upon exposure to light or heat during storage under the concurrent presence of the silver halide, organic silver salt and reducing agent which 40 remained in unexposed areas. It is contemplated that the presence of the reducing agent in the photothermographic material easily results in formation of fog upon reaction with the organic silver salt and that when exposed to light having different wavelengths from light employed in image recording after processing, the reducing agent functions as a 45 hole-trap in addition to its inherent function to reduce silver ions, leading to enhanced print-out from the silver halide or organic silver salt. In addition to the foregoing causes, it is contemplated that fog specs causing fogging are formed in 50 the course of manufacturing the photothermographic material.

A technique for solving these problems is disclosed in JP-A 6-208192 and 8-267934 (hereinafter, the term, JP-A means an unexamined and published Japanese Patent Application) and references cited therein. Although these disclosed techniques were effective to some extent, they 55 were not sufficiently at levels required by the market.

**SUMMARY OF THE INVENTION**

In view of the foregoing, the present invention was made 60 and it is therefore an object of the present invention to

provide a photothermographic material exhibiting little fogging even after storage for a long period of time and superior silver image stability after thermal processing.

The above object of the invention can be accomplished by 5 the following constitution:

1. A method for preparing a photothermographic material comprising an organic silver salt, wherein the method comprises a step of treating the organic silver salt under a gas atmosphere containing an inert gas having a volume fraction of not less than 85% or under a gas atmosphere containing oxygen gas having a volume fraction of not more than 15%;
2. The method described in 1, comprising the steps of:
  - (a) preparing an organic silver salt,
  - (b) preparing an emulsion containing the organic silver salt and a silver halide,
  - (c) drying the emulsion,
  - (d) coating the emulsion, and
  - (e) drying the coated emulsion,
 and wherein at least one of the steps (a) through (e) is conducted under the gas atmosphere containing an inert gas having a volume fraction of not less than 85% or under a gas atmosphere containing oxygen gas having a volume fraction of not more than 15%;
3. The method described in 2, wherein step (c) is conducted under the gas atmosphere containing an inert gas having a volume fraction of not less than 85% or under a gas atmosphere containing oxygen gas having a volume fraction of not more than 15%;
4. The method described in 1, wherein the inert gas is at least one selected from the group consisting of nitrogen, helium and argon;
5. The method described in 3, wherein in step (c), the emulsion is dried at a temperature of 35 to 80° C.;
6. The method described in 1, wherein the photothermographic material further comprises a light sensitive silver halide, a reducing agent and a binder;
7. The method described in 6, wherein the photothermographic material further comprises a cross-linking agent;
8. The method described in 7, wherein the photothermographic material further comprises a compound capable of generating a labile species other than a halogen atom upon exposure to ultraviolet ray or visible light to deactivate the reducing agent;
9. The method described in 8, wherein the labile species other than a halogen atom is a free radical comprised of plural atoms;
10. The method described in 7, wherein the cross-linking agent is selected from the group consisting of an epoxy compound, acid anhydride, an isocyanate compound, and an isothiocyanate compound;
11. A method of preparing a package containing a photothermographic material comprising an organic silver salt, wherein the method comprises a step of treating the organic silver salt under a gas atmosphere containing an inert gas having a volume fraction of not less than 85% or under a gas atmosphere containing oxygen gas having a volume fraction of not more than 15%;
12. The method described in 11, comprising the steps of:
  - (a) preparing an organic silver salt,
  - (b) preparing an emulsion containing the organic silver salt and a silver halide,
  - (c) drying the emulsion,
  - (d) coating the emulsion,

- (e) drying the coated emulsion to prepare a photothermographic material, and
- (f) packaging the photothermographic material to prepare a package containing the photothermographic material and wherein at least one of the steps (a) through (f) is conducted under the gas atmosphere containing an inert gas having a volume fraction of not less than 85% or under a gas atmosphere containing oxygen gas having a volume fraction of not more than 15%;
- 13. The method described in 12, wherein step (f) is conducted under the gas atmosphere containing an inert gas having a volume fraction of not less than 85% or under a gas atmosphere containing oxygen gas having a volume fraction of not more than 15%;
- 14. The method described in 11, wherein the inert gas is at least one selected from the group consisting of nitrogen, helium and argon;
- 15. The method described in 11, wherein the photothermographic material further comprises a light sensitive silver halide, a reducing agent and a binder;
- 16. A package containing a photothermographic material, wherein the package is filled with a gas containing an inert gas having a volume fraction of not less than 85% or with a gas containing oxygen gas having a volume fraction of not more than 15%;
- 17. The package described in 16, wherein the inert gas is at least one selected from the group consisting of nitrogen, helium, and argon;
- 18. The package of claim 16, wherein the package further contains a deoxidant;
- 19. The package described in 18, wherein the deoxidant is at least one selected from the group consisting of ferrous salts, iron powder, sulfites, hydrogen sulfites, dithionites, hydroquinone, catechol, resorcinol, pyrogallol, gallic acid, Rongalit, ascorbic acid, ascorbates, isoascorbic acid, isoascorbates, sorbose, glycose, lignin, dibutylhydroxytoluene, butylhydroxyanisole, and a mixture of the above-described oxygen absorbent and carbon dioxide absorbent, as described in JP-A No. 2-61148.

#### BRIEF EXPLANATION OF THE DRAWING

FIG. 1 illustrates a sectional view of a flash dryer used in the invention.

#### DETAILED DESCRIPTION OF THE INVENTION

The present invention will now be described in detail.

Examples of preferred inert gas usable in the process of preparing organic silver salts, the process of employing emulsions containing an organic silver salt and in packaging image recording/forming materials and specifically photothermographic materials include nitrogen gas, rare gases such as helium, neon and argon, and nitrogen gas is more preferred due to its low cost. Nitrogen gas obtained by vaporization of commercially available liquid nitrogen or commercially available cylinder nitrogen gas is preferred but one which is generated through chemical reaction is also usable. Further, it is preferred to employ copper chips, an aqueous ammonium carbonate solution, aqueous pyrogallol solution, vanadium sulfate solution, titanous salts and chromous salts to remove a trace amount of oxygen contained in nitrogen gas. Concrete methods are described in Jikken Kagaku Kohza (Series of Experimental Chemistry) vol. 5, pages 285-286.

One feature of this invention is to conduct the preparation process of an organic silver salt, dispersion of the emulsion

comprising an organic silver salt, silver halide and other additives and the drying process under an inert gas atmosphere or under a reduced oxygen-containing atmosphere. In such a case, the volume fraction of the inert gas is not less than 85%, and preferably not less than 95%. In other words, the inert gas preferably accounts for at least 85% by volume, and more preferably at least 95% by volume of the entire gas atmosphere. The total pressure of the atmosphere is preferably not less than normal atmospheric pressure. The volume fraction of oxygen is preferably not more than 15%, and more preferably not more than 5%. Effects of inert gas in this invention is remarkably displayed in cases when employed in the drying process of an organic silver salt-containing emulsion.

15 A gas atmosphere in the process of packaging image recording/forming materials and specifically, photothermographic materials is preferably the same as the foregoing. Further, it is preferred to introduce, after degassing under reduced pressure, a deoxidant into the package in an inert gas atmosphere under reduced pressure.

Deoxidants usable in the package relating to this invention are commonly known oxygen absorbents, including ferrous salts, iron powder, sulfites, hydrogen sulfites, dithionites, hydroquinone, catechol, resorcinol, pyrogallol, gallic acid, Rongalit, ascorbic acid, ascorbates, isoascorbic acid, isoascorbates, sorbose, glycose, lignin, dibutylhydroxytoluene, butylhydroxyanisole, and a mixture of the above-described oxygen absorbent and carbon dioxide absorbent, as described in JP-A No. 2-61148.

30 Packaging materials constituting a small gas-permeable bag usable as the deoxidant package include any one exhibiting gas-permeability of not more than 1000 sec/100 ml, based on Garley gas-permeability. Example thereof include paper such as Japanese paper, machine-made paper and rayon paper, non-woven fabric using various fibers such as pulp, cellulose or synthetic resin fiber, a packaging material laminated with perforated plastic resin film, paper and perforated polyethylene film and a packaging material of a fine porous membrane. Such deoxidant packages are known in the art, as described in JP-A Nos. 2-413, 2-61148, 2-12876, 2-182729 and 2-268806. A deoxidizing material in a sheet form is also usable, as described JP-A 2-86758.

Specifically, a lamination body which is comprised of 45 paper, an adhesive, a metal layer, an adhesive and a heat-sealing layer is preferred. In such an arrangement, even if paper or the metal layer is torn, the heat-sealing layer is not peeled off or cut, thereby leading to enhanced humidity resistance and light-tightness. Paper used for packaging material can be paper usually used for packaging, including non-bleached paper, bleached paper, art paper, coated paper and light coated paper. The thickness thereof is preferably 50 to 120 g/m<sup>2</sup>, and more preferably 70 to 95 g/m<sup>2</sup>. There may also be used additives to paper, such as a sizing agent, strength enhancing agent, and anti-foaming agent. Metals used for the metal layer are not specifically limited, including iron, aluminum, silver, and lead. Of these, aluminum is preferred. The metal is usually melted and extruded as a film, which may be used as a metallic foil (having a thickness of 5 to 25  $\mu$ m, and preferably 7 to 15  $\mu$ m). Metal powder may also be allowed to vapor-deposited on a plastic resin film. In this case, the thickness of the deposited membrane is preferably 8,000 to 18,000  $\text{\AA}$ .

In the heat-seal layer are used resins which are prepared 65 by polymerization using metallocene type catalysts. Exemplary examples thereof include polyolefinic resins such as high density polyethylene (HDPE), low density polyethyl-

ene (LDPE), linear low density polyethylene (LLDPE) and polypropylene (PP) and styrene type resins such as polystyrene. Metallocene is a compound having a structure in which a transitional metal is chelated by an unsaturated cyclic compound, and a combination of a Zr complex and methylaluminoxane (MAO) is well known. This catalyst is also called a Kaminsky catalyst or Kaminsky-Sinn catalyst. Injection molding is generally employed to manufacture film-molding products using resins prepared by the use of the metallocene catalyst. The injection molding method is not specifically limited, including conventional hot-runner type injection molding, metal mold vacuum injection and stack mold system. Of these, the hot-runner system is preferred. Various additives can be incorporated into the resin. Carbon black used for light-shielding preferably has a sulfur content of not more than 0.5% by weight to avoid adverse effects on photographic characteristics. Commercially available ones include, for example, #45 and #950 (a sulfur content of 0.5 and 0.4 wt %, respectively and produced by Mitsubishi Chemicals Co., Ltd), Bulcan (0.2 wt %, produced Gabott Corp.) and Denka Black (0.02 wt %, produced by DENKA Co., Ltd.). Carbon black is incorporated preferably in an amount of 0.3 to 0.6 wt %, and more preferably 0.35 to 0.40 wt %.

Enhanced physical properties and sufficient light-tightness can be achieved within this range. The heat-seal layer thickness is preferably 35 to 115  $\mu\text{m}$ . and more preferably 50 to 95  $\mu\text{m}$ . Among the metallocene type resins contained in the heat-seal layer, the content of a low molecular weight polymer is preferably not more than 8% by weight, and more preferably not more than 3% by weight. Further, the heat-seal layer may be added with an antistatic agent, a lubricant, an antioxidant or nucleating agent.

Various methods are applied to the method for laminating paper, a metal layer and a heat-seal layer through an adhesive. Examples thereof include an extruding inflation method, an extruding lamination method, and a dry lamination method, as described in Conver-Tech 1991, 1, "Lamination Shokyukoza (8)", page 10-14; Conver-Tech 1990, 5, "Lamination Shokyukoza (3)" page 40, 48; "Extrusion Molding of Plastic Resin and its Application" pages 137 and 147 (published by Seibundo); and "Plastic Handbook" page 727 (published by Asakura-shoten). In cases where carrying out lamination by the dry lamination method, the used adhesive can appropriately be selected from adhesives described in Conver-tech 1993, 3, "Lamination Shokyukoza (23)" pages 40 and 48. Of these, ester or urethane type adhesives are preferred, which have no adverse effect on photographic performance, such as fogging.

Lamination of the heat-seal layer over the metal layer via an adhesive is carried out at a temperature higher than the glass transition point ( $T_g$ ) of the heat-seal layer. The glass transition point ( $T_g$ ) is the temperature at which a liquid changes to an amorphous or glassy solid. The glass transition point of the heat-seal layer is preferably 50 to 150°C., and more preferably 75 to 95°C. The heat-seal layer can be formed by the extrusion laminating method or inflation laminating method. The formation is preferably carried out at a temperature higher than the glass transition temperature. Specifically, it was proved that forming the heat-seal layer by extrusion or inflation at 160 to 300°C. led to superior lateral lamination strength.

The metallocene type resin film prepared by extrusion or inflation is laminated with paper laminated with a metal foil

to form a packaging material, which is further supplied to a bag-making machine, wherein photographic materials are packaged by the center-pyro-sealing method or the three sided sealing method. Heat sealing may be carried out using a manual heat sealer. To prepare the package used in this invention, the photothermographic material may be loaded into an unsealed package under an inert gas atmosphere. Alternatively, after loading the photothermographic material, inert gas is introduced thereto and sealing is immediately conducted.

There can be employed various commonly known techniques for analysis of gas components contained in a gas atmosphere in the process of preparing organic silver salts, 15 the process of employing emulsions containing an organic silver salt and in packaging image recording/forming materials and specifically photothermographic materials or analysis of gas components contained in the package. Gas chromatography techniques generally used for analysis of inorganic gases are preferred, in which molecular sieves are 20 used as a filler for analysis of oxygen and nitrogen gases.

In this invention is also included a process for drying an 25 organic silver salt in the foregoing inert gas atmosphere at a temperature of 35 to 80°C., preferably 40 to 75°C., and more preferably 45 to 70°C. There is no specific limitation 30 with respect to a drying apparatus used in this invention and any kind of the apparatus can be used. Examples of preferred drying apparatus usable in this invention include a vacuum dryer, a freeze dryer, a hot air heating type tray dryer, a flash 35 dryer and a spray dryer, and the flash dryer is specifically preferred. The flash dryers include, for example, a straight pipe type, an expanded central barrel type for an increase of the retention time and a swing flow type, and the swing flow type is preferred. The flashing rate at the time of operating the flash dryer is preferably not less than 2.0  $\text{Nm}^3/\text{min}$ , more 40 preferably not less than 5.0  $\text{Nm}^3/\text{min}$ , and still more preferably not less than 8.0  $\text{Nm}^3/\text{min}$ . The hot air temperature is preferably not lower than 20°C., more preferably not lower than 40°C., and still more preferably not lower than 60°C.

An example of the flash dryer is shown in FIG. 1, as a 45 concrete apparatus meeting the object of the invention. FIG. 1 illustrates a cross section of an exemplary flash dryer used in this invention, in which drying and/or pulverization are carried out in the high-speed stream. In FIG. 1, numerals 1, 2 and 3 represent a hot air inlet, an inlet for slurry material and an inlet for wet cakes, respectively. Hot air heated to a prescribed temperature is blown through hot air inlet 1, using a fan. Slurry or wet cake containing an organic silver 50 salt is inputted through slurry inlet 2 or wet cake inlet 3, according to its wetting state, allowed to be transported through drying chamber 4 by high-speed air flow, passing through drying zone A and further passing via ascending section B through classification section C. Dried and undried 55 powders are classified, and dried powder alone passes via recovery section 5 through cyclone and bag-filter and recovered as powdery organic silver salt composition. Examples of concrete apparatus meeting the object of the invention include a flash jet dryer, available from Seishin Kogyo Co., 60 Ltd. Drying may be conducted two time in terms of productivity and prevention of over-drying.

As a reducing agent used in photothermographic materials are employed reducing agents containing a proton, such as bisphenols and sulfonamidophenols. Accordingly, a compound generating a labile species which is capable of abstracting a proton to deactivate the reducing agent is

preferred. More preferred is a compound as a non-colored photooxidizing substance, which is capable of generating a free radical as a labile species on exposure. Any compound having such a function is applicable. However, a halogen radical, which easily forms silver halide is not preferred. An organic free radical composed of plural atoms is preferred. Any compound having such a function and exhibiting no adverse effect on the photothermographic material is usable irrespective of its structure.

Of such free radical generation compounds, a compound containing an aromatic, and carbocyclic or heterocyclic group is preferred, which provides stability to the generated free radical so as to be in contact with the reducing agent for a period sufficient to react with the reducing agent to deactivate it. Representative examples of such compounds include biimidazolyl compounds and iodonium compounds. The imidazolyl compounds generate two imidazolyl radicals as a free radical upon exposure to ultraviolet or visible radiation, which are capable of oxidizing a reducing agent remaining after development, thereby inhibiting reduction of silver salts. It is surprising that the imidazolyl compound is photo-active and capable of oxidizing a reducing agent effective in heat-promoted reduction of a substantially non-photosensitive organic silver salt.

Of such imidazolyl compounds, a compound represented by the following formula [1] is preferred:

Formula [1]



wherein R<sub>1</sub>, R<sub>2</sub> and R<sub>3</sub> (which may be the same or different) each are an alkyl group (e.g., methyl, ethyl, hexyl), an alkenyl group (e.g., vinyl, allyl), an alkoxyl group (e.g., methoxy, ethoxy, octyloxy), an aryl group (e.g., phenyl, naphthyl, tolyl), hydroxy, a hydrogen atom, a halogen atom, an aryloxy (e.g., phenoxy), an alkylthio group (e.g., methythio, butylthio), an arylthio group (e.g., phenylthio), a heterocyclic group (e.g., pyridyl, triazyl), an acyl group (e.g., acetyl, propionyl, butyly, valeryl), a sulfonyl group (e.g., methylsulfonyl, phenylsulfonyl), an acylamino group, sulfonylamino group, an acyloxy group (e.g., acetoxy, benzoxy), carboxy, canyo, a sulfo group, or an amino group. Of these groups are preferred an aryl group, a heterocyclic group, an alkenyl group and cyano group.

The biimidazolyl compounds can be synthesized in accordance with the methods described in U.S. Pat. No. 3,734,733 and British Patent 1,271,177. Preferred Examples thereof are shown below.



|      | R <sub>1</sub>  | R <sub>2</sub> | R <sub>3</sub>  |
|------|-----------------|----------------|-----------------|
| BI-1 | H               | CN             | H               |
| BI-2 | CN              | H              | CN              |
| BI-3 | CF <sub>3</sub> | H              | CF <sub>3</sub> |
| BI-4 |                 |                |                 |
| BI-5 |                 |                |                 |
| BI-6 |                 |                |                 |
| BI-7 | H               |                | H               |
| BI-8 |                 |                |                 |
| BI-9 |                 |                |                 |



Similarly preferred compounds include a iodonium compound represented by the following formula (2):

Formula [2]



wherein R<sup>1</sup>, R<sup>2</sup>, R<sup>3</sup>, R<sup>4</sup>, X<sup>-</sup> and W are each the same as defined in formula [2]; Y is a carbon (i.e., —CH=) to form a benzene ring or a nitrogen atom (—N=) to form a pyridine ring.

The iodonium compounds described above can be synthesized in accordance with the methods described in Org. Syn., 1961 and Fieser, "Advanced Organic Chemistry" (Reinhold, N.Y., 1961). Examples of the suitable compounds are represented by the following general formulas.




---

| Compound | R <sup>1</sup>   | R <sup>2</sup>  | R <sup>3</sup>    | R <sup>4</sup>     | W | X                  | Y |
|----------|------------------|-----------------|-------------------|--------------------|---|--------------------|---|
| I-1      | H                | H               | H                 | OCOCH <sub>3</sub> | 1 | OCOCH <sub>3</sub> | C |
| I-2      | H                | H               | H                 | OCOCF <sub>3</sub> | 1 | OCOCF <sub>3</sub> | C |
| I-3      | H                | CH <sub>3</sub> | H                 | OCOCH <sub>3</sub> | 1 | OCOCH <sub>3</sub> | C |
| I-4      | H                | CH <sub>3</sub> | CO <sub>2</sub> H | O <sup>-</sup>     | 0 | —                  | C |
| I-5      | H                | H               | CO <sub>2</sub> H | O <sup>-</sup>     | 0 | —                  | C |
| I-6      | H                | CN              | CO <sub>2</sub> H | O <sup>-</sup>     | 0 | —                  | C |
| I-7      | OCH <sub>3</sub> | CH <sub>3</sub> | H                 | OCOCH <sub>3</sub> | 1 | OCOCH <sub>3</sub> | C |

-continued



| Compound | R <sup>1</sup>                                  | R <sup>2</sup>     | R <sup>3</sup>                | R <sup>4</sup>                     | W | X                                  | Y |
|----------|-------------------------------------------------|--------------------|-------------------------------|------------------------------------|---|------------------------------------|---|
| I-8      | CH <sub>3</sub>                                 | CH <sub>3</sub>    | CH <sub>3</sub>               | OCOCH <sub>3</sub>                 | 1 | OCOCH <sub>3</sub>                 | C |
| I-9      | CH <sub>3</sub>                                 | CH <sub>3</sub>    | H                             | OCOCH <sub>3</sub>                 | 1 | OCOCH <sub>3</sub>                 | C |
| I-12     | CH <sub>3</sub>                                 | CH <sub>3</sub>    | CO <sub>2</sub> H             | O <sup>-</sup>                     | 0 | —                                  | C |
| I-13     | H                                               | H                  | SO <sub>3</sub> H             | O <sup>-</sup>                     | 0 | —                                  | C |
| I-14     | H                                               | CN                 | CO <sub>2</sub> H             | O <sup>-</sup>                     | 0 | —                                  | C |
| I-15     | OCH <sub>3</sub>                                | Cl                 | H                             | OCOCH <sub>3</sub>                 | 1 | OCOCH <sub>3</sub>                 | C |
| I-16     | CO <sub>2</sub> H                               | H                  | H                             | OCOCH <sub>3</sub>                 | 1 | OCOCH <sub>3</sub>                 | C |
| I-17     | OCH <sub>3</sub>                                | Cl                 | CH <sub>3</sub>               | OCOCH <sub>3</sub>                 | 1 | OCOCH <sub>3</sub>                 | C |
| I-18     | H                                               | H                  | H                             | OCOCH <sub>2</sub> CH <sub>3</sub> | 1 | OCOCH <sub>2</sub> CH <sub>3</sub> | C |
| I-19     | H                                               | CH <sub>2</sub> OH | H                             | OCOCH <sub>3</sub>                 | 1 | OCOCH <sub>3</sub>                 | C |
| I-20     | Cl                                              | CH <sub>2</sub> OH | CO <sub>2</sub> H             | O <sup>-</sup>                     | 0 | —                                  | C |
| I-21     | Cl                                              | CH <sub>3</sub>    | SO <sub>3</sub> H             | O <sup>-</sup>                     | 0 | —                                  | C |
| I-22     | CH <sub>3</sub>                                 | CN                 | CO <sub>2</sub> H             | O <sup>-</sup>                     | 0 | —                                  | C |
| I-23     | CF <sub>3</sub>                                 | Cl                 | H                             | OCOCH <sub>3</sub>                 | 1 | OCOCH <sub>3</sub>                 | C |
| I-24     | CO <sub>2</sub> H                               | H                  | H                             | OCOCH <sub>3</sub>                 | 1 | OCOCH <sub>3</sub>                 | C |
| I-25     | OCC <sub>2</sub> H <sub>5</sub>                 | H                  | C <sub>6</sub> H <sub>5</sub> | OCOCH <sub>3</sub>                 | 1 | OCOCH <sub>3</sub>                 | C |
| I-26     | C <sub>6</sub> H <sub>5</sub>                   | H                  | H                             | OCOCH <sub>3</sub>                 | 1 | OCOCH <sub>2</sub> CH <sub>3</sub> | C |
| I-27     | C <sub>6</sub> H <sub>4</sub> CO <sub>2</sub> H | H                  | H                             | OCOCH <sub>3</sub>                 | 1 | OCOCH <sub>3</sub>                 | C |
| I-28     | H                                               | CH <sub>2</sub> OH | CO <sub>2</sub> H             | O <sup>-</sup>                     | 0 | —                                  | C |
| I-29     | SO <sub>2</sub> CH <sub>3</sub>                 | H                  | H                             | OCOCH <sub>3</sub>                 | 1 | OCOCH <sub>3</sub>                 | C |
| I-30     | Cl                                              | CN                 | CO <sub>2</sub> H             | O <sup>-</sup>                     | 0 | —                                  | C |
| I-31     | CF <sub>3</sub>                                 | OCH <sub>3</sub>   | H                             | OCOCH <sub>3</sub>                 | 1 | OCOCH <sub>3</sub>                 | C |
| I-32     | CO <sub>2</sub> H                               | CO <sub>2</sub> H  | H                             | OCOCH <sub>3</sub>                 | 1 | OCOCH <sub>3</sub>                 | C |
| I-33     | H                                               | H                  | H                             | OCOCH <sub>3</sub>                 | 1 | OCOCH <sub>3</sub>                 | N |
| I-34     | H                                               | H                  | H                             | OCOCF <sub>3</sub>                 | 1 | OCOCF <sub>3</sub>                 | N |
| I-35     | H                                               | COOH               | COOH                          | O <sup>-</sup>                     | 1 | OCOCH <sub>3</sub>                 | N |
| I-36     | H                                               | CN                 | COOH                          | O <sup>-</sup>                     | 0 | —                                  | N |
| I-37     |                                                 |                    |                               |                                    |   |                                    |   |



I-38



The compound releasing a labile species other than a halogen atom, such as represented by formula [1] or [2] is incorporated preferably in an amount of 0.001 to 0.1 mol/50 m<sup>2</sup>, and more preferably 0.005 to 0.05 mol/m<sup>2</sup>. The compound may be incorporated into any component layer of the photothermographic material relating to the invention and is preferably incorporated in the vicinity of a reducing agent.

As a compound capable of deactivating a reducing agent to inhibit reduction of an organic silver salt to silver by the reducing agent are preferred compounds releasing a labile species other than a halogen atom. However, these compounds may be used in combination with a compound capable of releasing a halogen atom as a labile species. The compound capable of releasing a halogen atom as a labile species is used preferably in an amount of 0.001 to 0.1 mol/m<sup>2</sup> and more preferably 0.005 to 0.05 mol/m<sup>2</sup>. Exemplary examples of the compound releasing an active halogen atom include a compound represented by the following formula [4]:



Formula [4]

55 wherein Q is an aryl group or a heterocyclic group; X<sub>1</sub>, X<sub>2</sub> and X<sub>3</sub> are each a hydrogen atom, a halogen atom, a haloalkyl group, an acyl group, an alkoxy carbonyl group, an aryloxycarbonyl group, a sulfonyl group, an aryl group or a heterocyclic group, provided that at least one of them is a halogen atom; Y is —C(=O)—, —SO— or —SO<sub>2</sub>—. The aryl group represented by Q may be a monocyclic or condensed ring group and is preferably a monocyclic or di-cyclic aryl group having 6 to 30 carbon atoms (e.g., phenyl, naphthyl), more preferably a phenyl or naphthyl group, and still more preferably a phenyl group. The heterocyclic group represented by Q is a 3- to 10-membered, saturated or unsaturated heterocyclic group containing at least one of N, O and S,

which may be a monocyclic or condensed with another ring to a condensed ring.

The heterocyclic group is preferably a 5- or 6-membered unsaturated heterocyclic group, which may be condensed, more preferably a 5- or 6-membered aromatic heterocyclic group, which may be condensed, still more preferably a N-containing 5- or 6-membered aromatic heterocyclic group, which may be condensed, and optimally a 5- or 6-membered aromatic heterocyclic group containing one to four N atoms, which may be condensed. Exemplary examples of heterocyclic rings included in the heterocyclic group include imidazole, pyrazole, pyridine, pyrimidine, pyrazine, pyridazine, triazole, triazines, indole, indazole, purine, thiazole, oxadiazole, quinoline, phthalazine, naphthyridine, quinoxaline, quinazoline, cinnoline, pteridine, acrydine, phenanthroline, phenazine, tetrazole, thiazole, oxazole, benzimidazole, benzoxazole, benzthiazole, indolenine and tetrazaindene. Of these are preferred imidazole, pyridine, pyrimidine, pyrazine, pyridazine, triazole, triazines, thiadiazole, oxadiazole, quinoline, phthalazine, naphthylizine, quinoxaline, quinazoline, cinnoline, tetrazole, thiazole, oxazole, benzimidazole, and tetrazaindene; more preferably imidazole, pyrimidine, pyridine, pyrazine, pyridazine, triazole, triazines, thiadiazole, quinoline, phthalazine, naphthyridine, quinoxaline, quinazoline, cinnoline, tetrazole, thiazole, benzimidazole, and benzthiazole; and still more preferably pyridine, thiazole, quinoline and benzthiazole.

The aryl group or heterocyclic group represented by Q may be substituted by a substituent, in addition to  $-\text{Y}-\text{C}$  30  $(\text{X}_1)(\text{X}_2)(\text{X}_3)$ . Preferred examples of the substituent include an alkyl group, an alkenyl group, an aryl group, an alkoxy group, an aryloxy group, an acyloxy group, an acyl group, an alkoxy carbonyl group, an aryloxy carbonyl group, an acyloxy group, an acylamino group, an alkoxy carbonyl amino group, an aryloxy carbonyl amino group, a sulfonyl amino group, a sulfamoyl group, a carbamoyl group, a sulfonyl group, a ureido group, phosphoramido group, a halogen atom, cyano group, sulfo group, carboxy group, nitro group and heterocyclic group. Of these are preferred an 40 alkyl group, an aryl group, an alkoxy group, an aryloxy group, an acyl group, an acylamino group, an aryloxy group, acyl group, an acylamino group, an alkoxy carbonyl group, an aryloxy carbonyl amino group, a sulfonamino group, a sulfamoyl group, a carbamoyl group, a ureido 45 group, phosphoramido group, a halogen atom, cyano group, nitro group, and a heterocyclic group; and more preferably an alkyl group, an aryl group, an alkoxy group, an aryloxy group, an acyl group, an acylamino group, a sulfonamino group, a sulfamoyl group, a carbamoyl group, a halogen 50 group, cyano group, nitro group and a heterocyclic group; and still more preferably an alkyl group, an aryl group and a halogen atom.  $\text{X}_1$ ,  $\text{X}_2$  and  $\text{X}_3$  are preferably a halogen atom, a haloalkyl group, an acyl group, an alkoxy carbonyl group, an aryloxy carbonyl group, a carbamoyl group, a sulfamoyl group, a sulfonyl group, and a heterocyclic group, more preferably a halogen atom, a haloalkyl group, an acyl group, an alkoxy carbonyl group, an acyl group, and a sulfonyl group, and still more preferably a halogen atom and a trihalomethyl group; and most preferably a halogen atom. 60 Of halogen atoms are preferably chlorine atom, bromine and iodine atom, and more preferably chlorine atom and bromine atom, and still more preferably bromine atom. Y is  $-\text{C}(=\text{O})-$ ,  $-\text{SO}-$ , and  $-\text{SO}_2-$ , and preferably  $-\text{SO}_2-$ .

Exemplary examples of these compounds are shown below.

4-1



4-2



4-3



4-4



4-5



4-6



4-7



4-8



4-9



4-10



4-11



4-12



**15**

-continued

**16**

-continued

4-13



4-14



4-15



4-16



4-17



4-18



4-19



4-20



4-21



4-22



4-23



60

4-24

4-25

4-26

4-27

4-28

4-29

4-30

4-31

4-32

4-33

4-34

**17**

-continued

**18**

-continued



19

-continued



20

These compounds are incorporated in an amount within a range such that increased formation of print-out silver produces substantially no problem, preferably in an amount of not more than 150%, and more preferably not more than 100% based on the compound releasing a labile species other than a halogen atom. As afore-mentioned, these compounds deactivate a reducing agent included in the thermally developable photosensitive layer, enhancing storage stability of the photothermographic material. Reducing agents used in the photothermographic materials and capable of deactivating a free radical will be described.

Reducing agents are incorporated into the photothermographic material of the present invention. Examples of suitable reducing agents are described in U.S. Pat. Nos. 3,770,448, 3,773,512, and 3,593,863, and Research Disclosure Items 17029 and 29963, and include the following: aminohydroxycycloalkenone compounds (for example, 2-hydroxypiperidino-2-cyclohexane); esters of amino reductones as the precursor of reducing agents (for example, piperidinohexose reducton monoacetate); N-hydroxyurea derivatives (for example, N-p-methylphenyl-N-hydroxyurea); hydrazones of aldehydes or ketones (for example, anthracenealdehyde phenylhydrazone; phosphamidophenols; phosphamidoanilines; polyhydroxybenzenes (for example, hydroquinone, t-butylhydroquinone, isopropylhydroquinone, and (2,5-dihydroxy-phenyl) methylsulfone); sulphydroxamic acids (for example, benzenesulphydroxamic acid); sulfonamidoanilines (for example, 4-(N-methanesulfonylona mide)aniline); 2-tetrazolylthiohydroquinones (for example, 2-methyl-5-(1-phenyl-5-tetrazolylthio)hydroquinone); tetrahydroquinoxalines (for example, 1,2,3,4-tetrahydroquinoxaline); amidoxines; azines (for example, combinations of aliphatic carboxylic acid arylhydrazides with ascorbic acid); combinations of polyhydroxybenzenes and hydroxylamines, reductones and/or hydrazine; hydroxamic acids; combinations of azines with sulfonamidophenols;  $\alpha$ -cyanophenylacetic acid derivatives; combinations of bis- $\beta$ -naphthol with 1,3-dihydroxybenzene derivatives; 5-pyrazolones, sulfonamidophenol reducing agents, 2-phenylindane-1,3-dione, etc.; chroman; 1,4-dihydropyridines (for example, 2,6-dimethoxy-3,5-dicarboethoxy-1,4-dihydropyridine); bisphenols (for example, bis(2-hydroxy-3-t-butyl-5-methylphenyl)methane, bis(6-hydroxy-m-tri)mesitol, 2,2-bis(4-hydroxy-3-methylphenyl)propane, 4,5-ethylidene-bis(2-t-butyl-6-methyl)phenol, UV-sensitive ascorbic acid derivatives and 3-pyrazolidones. Of these, particularly preferred reducing agents are hindered phenols. As hindered phenols, listed are compounds represented by the general formula (A) described below:

Formula (A)



wherein R represents a hydrogen atom or an alkyl group having from 1 to 10 carbon atoms (for example, isopropyl,  $-C_4H_9$ , 2,4,4-trimethylpentyl), and R' R'' each represents an alkyl group having from 1 to 5 carbon atoms (for example, methyl, ethyl, t-butyl).

Exemplary examples of the compounds represented by the formula (A) are shown below.



The used amount of reducing agents represented by the above-mentioned general formula (A) is preferably between  $1 \times 10^{-2}$  and 10 moles, and is more preferably between  $1 \times 10^{-2}$  and 1.5 moles per mole of silver.

- A-1 5 Silver halide emulsions used in the invention can be prepared according to the methods described in P. Glafkides, *Chimie Physique Photographique* (published by Paul Montel Corp., 19679; G. F. Duffin, *Photographic Emulsion Chemistry* (published by Focal Press, 1966); V. L. Zelikman et al., *Making and Coating of Photographic Emulsion* (published by Focal Press, 1964). Any one of acidic precipitation, neutral precipitation and ammoniacal precipitation is applicable and the reaction mode of aqueous soluble silver salt and halide salt includes single jet addition, double jet addition and a combination thereof. Specifically, preparation of silver halide grains with controlling the grain formation condition, so-called controlled double-jet precipitation is preferred. The halide composition of silver halide is not specifically limited and may be any one of silver chloride, silver chlorobromide, silver iodochlorobromide, silver bromide, silver iodobromide and silver iodide. After completing the grain formation, the resulting silver halide grain emulsion is subjected to desalting to remove soluble salts by commonly known washing methods such as a noodle washing method, a flocculation method, a ultrafiltration method, or electrodialysis to obtain desired emulsion grains.
- A-2 10 In order to minimize cloudiness after image formation and to obtain excellent image quality, the less the average grain size, the more preferred, and the average grain size is preferably not more than  $0.2 \mu\text{m}$ , more preferably between 0.01 and  $0.17 \mu\text{m}$ , and still more preferably between 0.02 and  $0.14 \mu\text{m}$ . The average grain size as described herein is defined as an average edge length of silver halide grains, in cases where they are so-called regular crystals in the form of cube or octahedron. Furthermore, in cases where grains are tabular grains, the grain size refers to the diameter of a circle having the same area as the projected area of the major faces. Furthermore, silver halide grains are preferably monodisperse grains. The monodisperse grains as described herein refer to grains having a coefficient of variation of grain size obtained by the formula described below of not more than 7%; more preferably not more than 5%, still more preferably not more than 3%, and most preferably not more than 1%.
- A-3 15 20 25
- A-4 30 35 40 45
- A-5 40 45
- A-6 50 55 60 65
- A-7 60 65
- 45 Coefficient of variation of grain size=standard deviation of grain diameter/average grain diameter $\times 100$  (%)

The grain form includes cubic, octahedral or tetradecahedral grains, tabular grains, spherical grains, bar-like grains, and potato-shaped grains. Of these, cubic grains, octahedral grains, tetradecahedral grains and tabular grains are specifically preferred.

The aspect ratio of tabular grains is preferably 2 to 100, and more preferably 3 to 50. These grains are described in U.S. Pat. Nos. 5,264,337, 5,314,798 and 5,320,958 and desired tabular grains can be readily obtained. Silver halide grains having rounded corners are also preferably employed.

The silver halide grain shape is not specifically limited, but a high ratio accounted for by a Miller index [100] plane is preferred. This ratio is preferably at least 50%; is more preferably at least 70%, and is most preferably at least 80%. The ratio accounted for by the Miller index [100] face can be obtained based on T. Tani, J. Imaging Sci., 29, 165 (1985) in which adsorption dependency of a [111] face or a [100] face is utilized.

It is preferred to use low molecular gelatin having an average molecular weight of not more than 50,000 in the

preparation of silver halide grains used in the invention, specifically, in the stage of nucleation. Thus, the low molecular gelatin has an average molecular weight of not more than 50,000, preferably 2,000 to 40,000, and more preferably 5,000 to 25,000. The average molecular weight can be determined by means of gel permeation chromatography. The low molecular gelatin can be obtained by subjecting an aqueous gelatin conventionally used and having an average molecular weight of ca. 100,000 to enzymatic hydrolysis, acid or alkali hydrolysis, thermal degradation at atmospheric pressure or under high pressure or ultrasonic degradation.

The concentration of dispersion medium used in the nucleation stage is preferably not more than 5% by weight, and more preferably 0.05 to 3.0% by weight.

In the preparation of silver halide grains, it is preferred to use a compound represent by the following formula [5], specifically in the nucleation stage:



Wherein Y is a hydrogen atom,  $-SO_3M$  or  $-CO-B-$  COOM, in which M is a hydrogen atom, alkali metal atom, ammonium group or ammonium group substituted by an alkyl group having carbon atoms of not more than 5, and B is a chained or cyclic group forming an organic dibasic acid; m and n each are 0 to 50, and p is 1 to 100. The compound represented by formula [5] has been employed as a defoaming agent to inhibit marked foaming occurred when stirring or moving emulsion raw materials, specifically in the stage of preparing an aqueous gelatin solution, adding a water-soluble silver and halide salts to the aqueous gelatin solution or coating an emulsion on a support during the process of preparing silver halide photographic light sensitive materials. A technique of using these compounds as a defoaming agent is described in JP-A 44-9497. The compound represented by formula [5] also functions as a defoaming agent during nucleation.

The compound represented by formula [5] is used preferably in an amount of not more than 1%, and more preferably 0.01 to 0.1% by weight, based on silver. The compound is to be present at the stage of nucleation, and may be added to a dispersing medium prior to or during nucleation. Alternatively, the compound may be added to an aqueous silver salt solution or halide solution used for nucleation. It is preferred to add it to a halide solution or both silver salt and halide solutions in an amount of 0.01 to 2.0% by weight. It is also preferred to make the compound represented by formula [5] present over a period of at least 50% (more preferably, at least 70%) of the nucleation stage. The compound may be added in the form of powder or solution using a solvent such as methanol. Representative examples of the compound represented by formula [5] are shown below, but are not limited to these.



-continued

E-4



E-5



E-6



The temperature during the stage of nucleation is preferably 5 to 60° C., and more preferably 15 to 50° C. Even when nucleation is conducted at a constant temperature, in a temperature-increasing pattern (e.g., in such a manner that nucleation starts at 25° C. and the temperature is gradually increased to reach 40° C. at the time of completion of nucleation) or its reverse pattern, it is preferred to control the temperature within the range described above.

Silver salt and halide salt solutions used for nucleation are preferably in a concentration of not more than 3.5N, and more preferably 0.01 to 2.5N. The flow rate of aqueous silver salt solution is preferably  $1.5 \times 10^{-3}$  to  $3.0 \times 10^{-1}$  mol/min per lit. of the solution, and more preferably  $3.0 \times 10^{-3}$  to  $8.0 \times 10^{-2}$  mol/min. per lit. of the solution. The pH during nucleation is within a range of 1.7 to 10, and since the pH at the alkaline side broadens the grain size distribution, the pH is preferably 2 to 6. The pBr during nucleation is 0.05 to 3.0, preferably 1.0 to 2.5, and more preferably 1.5 to 2.0.

Silver halide may be incorporated into an image forming layer by any means, in which silver halide is arranged so as to be as close to reducible silver source as possible. It is general that silver halide, which has been prepared in advance, added to a solution used for preparing an organic silver salt. In this case, preparation of silver halide and that of an organic silver salt are separately performed, making it easier to control the preparation thereof. Alternatively, as described in British Patent 1,447,454, silver halide and an organic silver salt can be simultaneously formed by allowing a halide component to be present together with an organic silver salt-forming component and by introducing silver ions thereto.

Silver halide can also be prepared by reacting a halogen containing compound with an organic silver salt through conversion of the organic silver salt. Thus, a silver halide-forming component is allowed to act onto a pre-formed organic silver salt solution or dispersion or a sheet material containing an organic silver salt to convert a part of the organic silver salt to photosensitive silver halide. The thus formed silver halide is effectively in contact with the organic silver salt, exhibiting favorable actions. In this case, the silver halide-forming component refers to a compound capable of forming silver salt upon reaction with the organic silver salt. Such a compound can be distinguished by the following simple test. Thus, a compound to be tested is to be mixed with the organic silver salt, and if necessary, the presence of a peak specific to silver halide can be confirmed by the X-ray diffractometry, after heating. Compounds that have been confirmed to be effective as a silver halide-forming component include inorganic halide compounds,

onium halides, halogenated hydrocarbons, N-halogeno compounds and other halogen containing compounds. These compounds are detailed in U.S. Pat. Nos. 4,009,039, 3,457,075 and 4,003,749, British Patent 1,498,956 and JP-A 53-27027 and 53-25420. Exemplary examples thereof are shown below:

- (1) Inorganic halide compound: e.g., a halide compound represented by formula,  $MX_n$ , in which M represents H, NH<sub>4</sub> or a metal atom; n is 1 when M is H or NH<sub>4</sub> and a number equivalent to a valence number of the metal atom when M is the metal atom; the metal atom includes lithium, sodium, potassium, cesium, magnesium, calcium, strontium, barium, zinc, cadmium, mercury, tin, antimony, chromium, manganese, cobalt, rhodium, and cerium, and molecular halogen such as aqueous bromine being also effective;
- (2) Onium halide: e.g., quaternary ammonium halides such as trimethylphenylammonium bromide, cetylethyldimethylammonium bromide, and trimethylbenzylammonium bromide; and tertiary sulfonium halides such as trimethylsulfonium iodide;
- (3) Halogenated hydrocarbons: e.g., iodoform, bromoform, carbon tetrachloride and 2-bromo-2-methylpropane;
- (4) N-halogeno compounds: e.g., N-chlorosuccinimide, N-bromosuccinimide, N-bromophthalimide, N-bromoacetoamide, N-iodosuccinimide, N-bromophthalazinone, N-bromoazolinone, N-chlorophthalazinone, N-bromoacetoanilide, N,N-dibromobenzenesulfonamide, N-bromo-N-methylbenzenesulfonamide, 1,3-dibromo-4,4-dimethylhydantoin and N-bromourazole;
- (5) Other halogen containing compounds: e.g., triphenylmethyl chloride, triphenylmethyl bromide 2-bromoacetic acid, 2-bromoethanol and dichlorobenzophenone.

The silver halide forming components may be used in combination. As described above, although silver halide can

be formed by converting a part or all of an organic silver salt to silver halide through reaction of the organic silver salt and a halide ion, it is preferred to use silver halide separately prepared which can be easily controlled with respect to grain size or grain form. The silver halide separately prepared may be used in combination with silver halide prepared by conversion of at least a part of an organic silver salt. The silver halide which is separately prepared or prepared through conversion of an organic silver salt is used preferably in an amount of 0.001 to 0.7 mol, and more preferably 0.03 to 0.5 mol per mol of organic silver salt.

Silver halide preferably occludes ions of metals belonging to Groups 6 to 11 of the Periodic Table. Preferred as the metals are W; Fe, Co, Ni, Cu, Ru, Rh, Pd, Re, Os, Ir, Pt and Au. These metals may be introduced into silver halide in the form of a complex.

The photosensitive silver halide grains used in the invention is preferably subjected to a chemical sensitization. As preferable chemical sensitizations, well known chemical sensitizations in this art such as a sulfur sensitization, a selenium sensitization and a tellurium sensitization are usable. Furthermore, a noble metal sensitization using gold, platinum, palladium and iridium compounds and a reduction sensitization are available.

Silver halide used in the invention is preferably spectral-sensitized by allowing a sensitizing dye to adsorb onto the silver halide. Useful sensitizing dyes used in the invention are also described in RD17643, sect. IV-A (December, 1978, page 23) and RD18431 sect. IX (August, 1978, page 437). It is specifically preferred to use sensitizing dyes exhibiting spectral sensitivity suited for spectral characteristics of light sources used in a laser imager or a scanner, as described in JP-A 9-34078, 9-54409 and 9-80679.

It is specifically preferred to use sensitizing dyes exhibiting sensitivity to the infrared region. Examples of preferred infrared sensitizing dyes used in the invention include those described in U.S. Pat. Nos. 4,536,473, 4,515,888 and 4,959,294.

Specifically, preferred sensitizing dyes are dyes represented by the following formulas (1) to (4):

Formula (1)



Formula (2)



-continued

Formula (3)



Formula (4)



In formulas (1) to (4),  $Y_1$ ,  $Y_2$ ,  $Y_{11}$ ,  $Y_{21}$ ,  $Y_{22}$  and  $Y_{31}$  each are independently an oxygen atom, a sulfur atom, a selenium atom,  $—C(Ra)(Rb)—$  group or  $—CH=CH—$  group, in which Ra and Rb each are a hydrogen atom, an alkyl group (preferably having 1 to 5 carbon atoms) or a non-metallic atom group necessary to form an aliphatic spiro ring;  $Z_1$  is a non-metallic atom group necessary to form a 5- or 6-membered ring;  $R_1$ ,  $R_{11}$ ,  $R_{21}$ ,  $R_{22}$ ,  $R_{31}$  and  $R_{32}$  each are an aliphatic group or a non-metallic atom group necessary to form a condensed ring between  $R_1$  and  $W_3$  or between  $R_{11}$  and  $W_{14}$ ;  $Rc$  and  $Rd$  each are independently an unsubstituted lower alkyl group, a cycloalkyl group, an aralkyl group, an aryl group or a heterocyclic group;  $W_1$ ,  $W_2$ ,  $W_3$ ,  $W_4$ ,  $W_{11}$ ,  $W_{12}$ ,  $W_{13}$ ,  $W_{14}$ ,  $W_{21}$ ,  $W_{22}$ ,  $W_{23}$ ,  $W_{24}$ ,  $W_{31}$ ,  $W_{32}$ ,  $W_{33}$  and  $W_{34}$  each are independently a hydrogen atom, a substituent or a non-metallic atom group necessary to form a condensed ring by bonding between  $W_1$  and  $W_2$ ,  $W_{11}$ , and  $W_{12}$ ,  $W_{21}$  and  $W_{22}$ ,  $W_{23}$  and  $W_{24}$ ,  $W_{31}$  and  $W_{32}$ , or  $W_{33}$  and  $W_{34}$ ;  $V_1$  to  $V_9$ ,  $V_{11}$  to  $V_{13}$ ,  $V_{21}$ , to  $V_{29}$ , and  $V_{31}$  to  $V_{33}$  each are independently a hydrogen atom, a halogen atom, an amino group, an alkylthio group, an arylthio group, a lower alkyl group, a lower alkoxy group, an aryl group, an aryloxy group, a heterocyclic group or a non-metallic atom group necessary to form a 5- to 7-membered ring by bonding between  $V_1$  and  $V_3$ ,  $V_2$  and  $V_4$ ,  $V_3$  and  $V_5$ ,  $V_2$  and  $V_6$ ,  $V_5$  and  $V_7$ ,  $V_6$  and  $V_8$ ,  $V_7$  and  $V_9$ ,  $V_{11}$  and  $V_{13}$ ,  $V_{21}$  and  $V_{23}$ ,  $V_{22}$  and  $V_{24}$ ,  $V_{23}$  and  $V_{25}$ ,  $V_{24}$  and  $V_{26}$ ,  $V_{25}$  and  $V_{27}$ ,  $V_{26}$  and  $V_{28}$ ,  $V_{27}$  and  $V_{29}$ , or  $V_{31}$  and  $V_{33}$ ;  $X_{21}$  and  $X_{31}$ , provided that at least one of  $V_1$  to  $V_9$  and at least one of  $V_{11}$  to  $V_{13}$  are a group other than a hydrogen atom;  $X_1$ ,  $X_{11}$ ,  $X_{21}$  and  $X_{31}$  each are an ion necessary to compensate for an intramolecular charge; 11, 111, 121 and 131 each an ion necessary to compensate for an intramolecular charge;  $k1$ ,  $k2$ ,  $k31$  and  $k32$  each are 0 or 1;  $n21$ ,  $n22$ ,  $n31$  and  $n32$  each are 0, 1 or 2; provided that  $n1$  and  $n22$ , and  $n31$  and  $n32$  are not 0 at the same time;  $p1$  and  $p11$  are each 0 or 1;  $q1$  and  $q11$  each are 1 or 2, provided that the sum of  $p1$  and  $q1$  and the sum of  $p11$  and  $q11$  each are respectively not more than 2.

Of formulas (1) and (2), a compound represented by the following formula (1-1) or (2-1) is more preferred:



Formula (1-1)



Formula (2-1)

wherein  $Y_1$ ,  $Y_2$  and  $Y_{11}$  each are independently an oxygen atom, a sulfur atom, a selenium atom,  $—C(Ra)(Rb)—$  group or  $—CH=CH—$  group, in which Ra and Rb each are a hydrogen atom, a lower alkyl group or an atomic group necessary to form an aliphatic spiro ring when Ra and Rb are linked with each other;  $Z_1$  is an atomic group necessary to form a 5- or 6-membered ring; R is a hydrogen atom, a lower alkyl, a cycloalkyl group, an aralkyl group, a lower alkoxy group, an aryl group, a hydroxy group or a halogen atom;  $W_1$ ,  $W_2$ ,  $W_3$ ,  $W_4$ ,  $W_{11}$ ,  $W_{12}$ ,  $W_{13}$  and  $W_{14}$  each are independently a hydrogen atom, a substituent or a non-metallic atom group necessary to form a condensed ring by bonding between  $W_1$  and  $W_2$  or  $W_{11}$  and  $W_{12}$ ;  $R_1$  and  $R_{11}$  are each an aliphatic group or a non-metallic atom group necessary to form a condensed ring by bonding between  $R_1$  and  $W_3$  or  $R_{11}$  and  $W_{14}$ ;  $L_1$  to  $L_9$ , and  $L_{11}$  to  $L_{15}$  each are independently a methine group;  $X_1$  and  $X_{11}$  each are an ion necessary to compensate for an intramolecular charge; 11 and 111 each an ion necessary to compensate for an intramolecular charge;  $k1$  and  $k2$  each are 0 or 1;  $p1$  and  $p11$  are each 0 or 1;  $q1$  and  $q11$  each are 1 or 2, provided that the sum of  $p1$  and  $q1$  and the sum of  $p11$  and  $q11$  each are respectively not more than 2.

Exemplary examples of the sensitizing dyes represented by formulas (1), (1-1), (2-1), (3) and (4) are shown below, but are not limited to these.

Compound represented by Formulas (1) to (4):

No. S-1



No. S-2



No. S-3



No. S-4



No. S-5



No. S-6







**35**

-continued

**36**

No. S-21



No. S-22



No. S-23



No. S-24



No. S-25



No. S-26



-continued



No. S-27



No. S-28



No. S-29



No. S-30



No. S-31



No. S-32



No. S-33



-continued

No. S-41



No. S-42



No. S-43



No. S-44



No. S-45



No. S-46



No. S-47



No. S-48



-continued

No. S-49



No. S-50



No. S-51



No. S-52



No. S-53



No. S-54



No. S-55





-continued



No. S-63



No. S-64



No. S-65



No. S-66



No. S-67



No. S-68

-continued

No. S-69



No. S-70



The infrared sensitizing dyes and spectral sensitizing dyes described above can be readily synthesized according to the methods described in F. M. Hammer, *The Chemistry of Heterocyclic Compounds* vol.18, "The cyanine Dyes and Related Compounds" (A. Weissberger ed. Interscience Corp., New York, 1964).

These sensitizing dyes may be used alone or in combination thereof. The combined use of sensitizing dyes is often employed for the purpose of supersensitization. A supersensitizing compound, such as a dye which does not exhibit spectral sensitization or substance which does not substantially absorb visible light may be incorporated, in combination with a sensitizing dye, into the emulsion.

In cases when being super-sensitized, and specifically when a reducing agent is not deactivated, photosensitivity is enhanced, print-out is easily promoted after development. In such a case, the present invention is effective. In cases when being infrared-sensitized, an infrared sensitizing dye has an oxidation-reduction potential at which a silver halide or an organic silver salt is slightly reducible, easily producing a silver cluster forming fog silver in the presence of the reducing agent, even when placed in a dark room. The produced silver cluster also induces fogging as a catalyst nucleus, deteriorating storage stability in the dark room or promoting print-out when placed in a daylight room after development. Further, sensitivity of the infrared sensitive material extends to the thermal radiation region outside the visible region so that the present invention is effective for inhibiting print-out silver produced by thermal radiation. Such a effect is marked in infrared-sensitized photosensitive materials which is sensitized with a supersensitizer. Useful sensitizing dyes, dye combinations exhibiting supersensitization and materials exhibiting supersensitization are described in RD17643 (published in December, 1978), IV-J at page 23, JP-B 9-25500 and 43-4933 (herein, the term, JP-B means published Japanese Patent) and JP-A 59-19032, 59-192242 and 5-341432.

In the invention, an aromatic heterocyclic mercapto compound represented by the following formula (6) is preferred as a supersensitizer:

### Ar—SM

Formula (6)

wherein M is a hydrogen atom or an alkali metal atom; Ar is an aromatic ring or condensed aromatic ring containing a

25 nitrogen atom, oxygen atom, sulfur atom, selenium atom or tellurium atom. Such aromatic heterocyclic rings are preferably benzimidazole, naphthoimidazole, benzthiazole, naphthothiazole, benzoxazole, naphthooxazole, benzoselenazole, benzotellurazole, imidazole, oxazole, 30 pyrazole, triazole, triazines, pyrimidine, pyridazine, pyrazine, pyridine, purine, and quinoline. Other aromatic heterocyclic rings may also be included.

A disulfide compound which is capable of forming a mercapto compound when incorporated into a dispersion of an organic silver salt and/or a silver halide grain emulsion is also included in the invention. In particular, a preferred example thereof is a disulfide compound represented by the following formula:

$$\text{Ar}-\text{S}-\text{S}-\text{Ar}$$

Formula (7)

<sup>40</sup> wherein Ar is the same as defined in formula (6)

The aromatic heterocyclic rings described above may be substituted with a halogen atom (e.g., Cl, Br, I), a hydroxy group, an amino group, a carboxy group, an alkyl group (having one or more carbon atoms, and preferably to 4 carbon atoms) or an alkoxy group (having one or more carbon atoms, and preferably to 4 carbon atoms).

Exemplary examples of mercapto-substituted aromatic heterocyclic compound are shown below but are not limited to these.

50 M-1: 2-mercaptopbenzimidazole  
M-2: 2-mercaptopbenzoxazole  
M-3: 2-mercaptopbenzthiazole  
55 M-4: 5-methyl-2-mercaptopbenzimidazole  
M-5: 6-ethoxy-2-mercaptopbenzthiazole  
M-6: 2,2'-dithiobis(benzthiazole)  
M-7: 3-mercaptop-1,2,4-triazole  
M-8: 4,5-diphenyl-2-imidazole  
60 M-9: 2-mercaptopimidazole  
M-10: 1-ethyl-2-mercaptopbenzimidazole  
M-11: 2-mercaptopquinoline  
M-12: 8-mercaptopurine  
65 M-13: 2-mercaptop-4(3H)-quinazoline  
M-14: 7-trifluoromethyl-4-quinolinethiol  
M-15: 2,3,5,6-tetrachloro-4-pyridinethiol

- M-16: 4-amino-6-hydroxy-2-mercaptopypyridine monohydrate  
 M-17: 2-amino-5-mercaptop-1,3,4-thiazole  
 M-18: 3-amino-5-mercaptop-1,2,4-triazole  
 M-19: 4-hydroxy-2-mercaptopypyridine  
 M-20: 2-mercaptopypyridine  
 M-21: 4,6-diamino-2-mercaptopypyridine  
 M-22: 2-mercaptop-4-methylpyrimidine hydrochloride  
 M-23: 3-mercaptop-5-phenyl-1,2,4-riazole  
 M-24: 2-mercaptop-4-phenyloxazole

The supersensitizer compound usable in the invention is incorporated into an emulsion layer containing the organic silver salt and silver halide grains, preferably in an amount of 0.001 to 1.0 mol, and more preferably 0.01 to 0.5 mol per mol of silver.

Binders suitable for the photothermographic material to which the present invention is applied are transparent or translucent, and generally colorless. Binders are natural polymers, synthetic resins, and polymers and copolymers, other film forming media; for example, gelatin, gum arabic, poly(vinyl alcohol), hydroxyethyl cellulose, cellulose acetate, cellulose acetatebutylate, poly(vinylpyrrolidone), casein, starch, poly(acrylic acid), poly(methylmethacrylic acid), poly(vinyl chloride), poly(methacrylic acid), copoly(styrene-maleic acid anhydride), copoly(styrene-acrylonitrile), copoly(styrene-butadiene), poly(vinyl acetal) series (for example, poly(vinyl formal) and poly(vinyl butyral), poly(ester) series, poly(urethane) series, phenoxy resins, poly(vinylidene chloride), poly(epoxide) series, poly(carbonate) series, poly(vinyl acetate) series, cellulose esters, poly(amide) series. These may be hydrophilic or hydrophobic polymers. of these, as a binder preferable for the thermally developable photosensitive layer is polyvinyl acetals and more preferably polyvinyl butyral. Cellulose esters exhibiting higher softening temperature, such as triacetyl cellulose or cellulose acetatebutylate are preferred for non-photosensitive layers such as an over-coat layer or sub-coat layer, specifically, a protective layer or backing layer. These binders may be used in combination. The binder is used with a range effective to function as a binder. The effective range can optimally be determined by one skilled in the art. As a measure to hold at least an organic silver salt, a ratio of a binder to an organic silver salt, based on weight is preferably within a range of 15:1 to 1:2, more preferably 8:1 to 1:1. The amount of a binder in a photosensitive layer is preferably 1.5 to 6 g/m<sup>2</sup>, and more preferably 1.7 to 5 g/m<sup>2</sup>. The amount of less than 1.5 g/m<sup>2</sup> results in an increase density of an unexposed area to levels unacceptable to practical use.

Inclusion of a cross-linking agent is specifically effective in the invention. Although the mechanism has not been elucidated, it was proved that the combined use of the cross-linking agent and the labile species-generating compound used relating to the invention gave advantageous effects on storage stability on the dark room and production of print-out silver under daylight. Although it is commonly known that the use of a cross-linking agent in such a binder as described above improves layer adhesion and lessens unevenness in development, it is unexpected that the use of the crosslinking agent in combination with the labile species-generating compound was effective in fog inhibition during storage and prevention of print-out after development.

Crosslinking agents usable in the invention include various commonly known crosslinking agents used for photographic materials, such as aldehyde type, epoxy type, vinyl-

sulfon type, sulfonester type, acryloyl type, carbodiimide type crosslinking agents, as described in JP-A 50-96216. Specifically preferred are an isocyanate type compound, epoxy compound and acid anhydride, as shown below.

5 One of the preferred crosslinking agents is an isocyanate or thioisocyanate compound represented by the following formula:



10 wherein v is 1 or 2; L is a bivalent linkage group of an alkylene, alkenylene, arylene or alkylarylene group; and X is an oxygen atom or a sulfur atom. An arylene ring of the arylene group may be substituted. Preferred substituents include a halogen atom (e.g., bromine atom, chlorine atom), hydroxy, amino, carboxy, alkyl and alkoxy.

15 The isocyanate crosslinking agent is an isocyanate compound containing at least two isocyanate group and its adduct. Examples thereof include aliphatic isocyanates, alicyclic isocyanates, benzeneisocyanates, naphthalenediisocyanates, biphenyldiisocyanates, diphenylmethandiisocyanates, triphenylmethanediisocyanates, triisocyanates, tetraisocyanates, their adducts and adducts of these isocyanates and bivalent or trivalent polyhydric alcohols. Exemplary examples are isocyanate compounds described in JP-A 56-5535 at pages 10-12. Of these, adduct of an isocyanate and polyvinyl alcohol enhanced interlayer adhesion and prevents peeling of a layer, image doubling and generation of bubbles

20 The thioisocyanate type crosslinking agent usable in the invention is to be a compound having a thioisocyanate structure, corresponding to the isocyanates described above.

25 30 The crosslinking agents described above are used preferably in an amount of 0.001 to 2 mol, and more preferably 0.005 to 0.5 mol per mol of silver.

35 The epoxy compound usable in the invention may be any one containing at least one epoxy group and is not limited 40 with respect to the number of the epoxy group, molecular weight and other parameters. The epoxy group is preferably contained in the form of a glycidyl group through an ether bond or an imino bond in the molecule. The epoxy compound may be any one of a monomer, oligomer and polymer, 45 in which the number of the epoxy group in the molecule is preferably 1 to 10 and more preferably 2 to 4. In cases where the epoxy compound is a polymer, it may be either one of a homopolymer and a copolymer. The number-averaged molecular weight (Mn) thereof is preferably 2,000 to 50 20,000. The amount to be added is not specifically limited, but preferably  $1 \times 10^{-6}$  to  $1 \times 10^{-2}$  mol/m<sup>2</sup>, and more preferably  $1 \times 10^{-5}$  to  $1 \times 10^{-3}$  mol/m<sup>2</sup>.

55 The acid anhydride used in the invention is preferably a compound containing at least an acid anhydride group represented as below:



60 65 The acid anhydride usable in the invention may be any compound containing one or more acid anhydride group, the number of the acid anhydride group, molecular weight or other parameters are not specifically limited.

Exemplary examples of the acid anhydride compound are shown below but are not limited to these.

**53****54**

-continued

B-9

B-1



B-2 10



B-10



B-3 20



B-11



B-4



B-12



B-5



B-13



B-6 45



B-14



B-7



B-15



B-8 60



65

55

-continued



B-16



B-17

The acid anhydride compound may be used alone or combination thereof. The amount to be added is not specifically limited, but preferably  $1 \times 10^{-6}$  to  $1 \times 10^{-1}$  mol/m<sup>2</sup>, and more preferably  $1 \times 10^{-4}$  to  $1 \times 10^{-2}$  mol/m<sup>2</sup>.

The cross-linking agent may be added to any layer of a photosensitive layer, surface protective layer, interlayer, antihalation layer and subbing layer provided on the photosensitive layer-side of the support and may be added to one or plurality of these layers. Further, it may be added to a layer provided on the opposite side of the support, in combination with the photosensitive layer-side. In the case of a photothermographic material having photosensitive layers on both sides of the support, it may be added to any one of the layers.

Organic silver salts used in the invention are reducible silver source, and silver salts of organic acids or organic heteroacids are preferred and silver salts of long chain fatty acid (preferably having 10 to 30 carbon atom and more preferably 15 to 25 carbon atoms) or nitrogen containing heterocyclic compounds are more preferred. Specifically, organic or inorganic complexes, ligand of which have a total stability constant to a silver ion of 4.0 to 10.0 are preferred. Exemplary preferred complex salts are described in RD17029 and RD29963, including organic acid salts (for example, salts of gallic acid, oxalic acid, behenic acid, stearic acid, palmitic acid, lauric acid, etc.); carboxyalkylthiourea salts (for example, 1-(3-carboxypropyl)thiourea, 1-(3-carboxypropyl)-3,3-dimethylthiourea, etc.); silver complexes of polymer reaction products of aldehyde with hydroxy-substituted aromatic carboxylic acid (for example,

56

- aldehydes (formaldehyde, acetaldehyde, butyraldehyde, etc.), hydroxy-substituted acids (for example, salicylic acid, benzoic acid, 3,5-dihydroxybenzoic acid, 5,5-thiodisalicylic acid, silver salts or complexes of thiones (for example, 5-3-(2-carboxyethyl)-4-hydroxymethyl-4-(thiazoline-2-thione and 3-carboxymethyl-4-thiazoline-2-thione), complexes of silver with nitrogen acid selected from imidazole, pyrazole, urazole, 1,2,4-thiazole, and 1H-tetrazole, 3-amino-5-benzylthio-1,2,4-triazole and benztriazole or salts thereof; 10 silver salts of saccharin, 5-chlorosalicylaldoxime, etc.; and silver salts of mercaptides. Of these organic silver salts, silver salts of fatty acids are preferred, and silver salts of behenic acid, arachidinic acid and stearic acid are specifically preferred.
- 15 The organic silver salt compound can be obtained by mixing an aqueous-soluble silver compound with a compound capable of forming a complex. Normal precipitation, reverse precipitation, double jet precipitation and controlled double jet precipitation described in JP-A 9-127643 are 20 preferably employed. For example, to an organic acid is added an alkali metal hydroxide (e.g., sodium hydroxide, potassium hydroxide, etc.) to form an alkali metal salt soap of the organic acid (e.g., sodium behenate, sodium arachidinate, etc.), thereafter, the soap and silver nitrate are 25 mixed by the controlled double jet method to form organic silver salt crystals. In this case, silver halide grains may be concurrently present.

In the present invention, organic silver salts have an average grain diameter of 10  $\mu\text{m}$  or less and are monodisperse. The average diameter of the organic silver salt as described herein is, when the grain of the organic salt is, for example, a spherical, cylindrical, or tabular grain, a diameter of the sphere having the same volume as each of these grains. The average grain diameter is preferably between 30 0.05 and 10  $\mu\text{m}$ , more preferably between 0.05 and 5  $\mu\text{m}$  and still more preferably between 0.05 and 0.5  $\mu\text{m}$ . Furthermore, the monodisperse as described herein is the same as silver halide grains and preferred monodispersibility is between 1 and 30%.

35 It is also preferred that at least 60% of the total of the organic silver salt is accounted for by tabular grains. The tabular grains refer to grains having a ratio of an average grain diameter to grain thickness, i.e., aspect ratio (denoted as AR) of 3 or more:

$$45 \text{ AR} = \text{diameter } (\mu\text{m}) / \text{thickness } (\mu\text{m})$$

To obtain such tabular organic silver salts, organic silver salt crystals are pulverized together with a binder or surfactant, using a ball mill. Thus, using these tabular grains, photosensitive materials exhibiting high density and superior image fastness are obtained.

50 To prevent hazing of the photosensitive material, the total amount of silver halide and organic silver salt is preferably 0.5 to 2.2 g in equivalent converted to silver per m<sup>2</sup>, thereby leading to high contrast images.

The photothermographic material (hereinafter, also referred to as photothermographic material), which forms images upon thermal development, comprises a reducible silver source (such as an organic silver salt), photosensitive silver halide, reducing agent and optionally an image toning agent to modify silver image color, which are dispersed in an (organic) binder matrix. The photothermographic material is stable at ordinary temperatures, which is developed, after exposure, upon heating at a high temperature (e.g., 80 to 140° C.). On heating, silver is formed through oxidation-reduction reaction between the organic silver salt (which acts as an oxidant) and the reducing agent. The oxidation-

reduction reaction is catalyzed by silver latent images formed upon exposure to light. Silver formed by reaction of the organic silver salt in exposed areas provides a black image in contrast to non-exposed areas, forming images. This reaction process proceeds without supplying processing solution such as water from the exterior.

Image toning agents are preferably incorporated into the photothermographic material used in the present invention. Examples of preferred image toning agents are disclosed in Research Disclosure Item 17029. Further, the photothermographic materials used in this invention may contain anti-foggants.

In the photothermographic material used in this invention, a matting agent is preferably incorporated into the image forming layer side. In order to minimize the image abrasion after thermal development, the matting agent is provided on the surface of a photosensitive material and the matting agent is preferably incorporated in an amount of 0.5 to 30 per cent in weight ratio with respect to the total binder in the emulsion layer side.

In cases where a non photosensitive layer is provided on the opposite side of the support to the photosensitive layer, it is preferred to incorporate a matting agent into at least one of the non-photosensitive layer (and more preferably, into the surface layer) in an amount of 0.5 to 40% by weight, based on the total binder on the opposite side to the photosensitive layer.

Materials of the matting agents employed in the present invention may be either organic substances or inorganic substances.

The shape of the matting agent may be crystalline or amorphous. However, a crystalline and spherical shape is preferably employed. The size of a matting agent is expressed in the diameter of a sphere having the same volume as the matting agent. The particle diameter of the matting agent in the present invention is referred to the diameter of a spherical converted volume. The matting agent employed in the present invention preferably has an average particle diameter of 0.5 to 10  $\mu\text{m}$ , and more preferably of 1.0 to 8.0  $\mu\text{m}$ . Furthermore, the variation coefficient of the size distribution is preferably not more than 50%, is more preferably not more than 40%, and is most preferably not more than 30%.

In addition to these materials, a variety of additives may be optionally incorporated into the photosensitive layer, non-photosensitive layer or other component layer(s). The photothermographic materials of the invention may be added with a surfactant, an antioxidant, a stabilizer, a plasticizer, a UV absorbent or a coating aid. As these additives and other additives described above are preferably employed compounds described in RD17029 (June, 1978, pages 9 to 15).

Supports usable in the photothermographic materials include various kinds of polymeric materials, glass, wool fabric, cotton fabric, paper, metal (e.g., aluminum) and those which are convertible to flexible sheets or rolls are preferred in terms of handling as information recording material. Preferred supports usable in photothermographic materials are plastic resin films (e.g., cellulose acetate film, polyester film, polyethylene terephthalate film, polyethylene naphthalate film, polyamide film, polyimide film, cellulose triacetate film, polycarbonate film) and biaxially stretched polyethylene terephthalate film is specifically preferred. The thickness of the support is preferably 50 to 300  $\mu\text{m}$ , and more preferably 70 to 180  $\mu\text{m}$ .

In the present invention, to improve an electrification property, a conducting compound such as a metal oxide and/or a conducting polymer can be incorporated into a construction layer. These compounds can be incorporated

into any layer, preferably into a sublayer, a backing layer and an intermediate layer between a photosensitive layer and a sublayer, etc. In the present invention, the conducting compounds described in U.S. Pat. No. 5,244,773, column 14 through 20, are preferably used.

The coating method of the photosensitive layer, protective layer and backing layer is not specifically limited. Coating can be conducted by any method known in the art, including air knife, dip-coating, bar coating, curtain coating, and hopper coating. Two or more layers can be simultaneously coated. As a solvent for coating solution are employed organic solvents such as methyl ethyl ketone (also denoted as MEK), ethyl acetate and toluene.

The photothermographic material according to the invention comprises a support having thereon a photosensitive layer, and preferably further on the photosensitive layer having a non-photosensitive layer. For example, it is preferred that a protective layer is provided on the photosensitive layer to protect the photosensitive layer and that a back coating layer is provided on the opposite side of the support to the photosensitive layer to prevent adhesion between photosensitive materials or sticking of the photosensitive material to a roller. Further, there may be provided a filter layer on the same side or opposite side to the photosensitive layer to control the amount or wavelengths of light transmitting the thermally developable photosensitive layer. Alternatively, a dye or pigment may be incorporated into the photosensitive layer. In this case, dyes described in JP-A 8-201959 are preferably used therein. The photosensitive layer may be comprised of plural layers. To adjust contrast, a high-speed layer and low speed layer may be provided in combination. Various adjuvants may be incorporated into the photosensitive layer, non-photosensitive layer or other component layer(s).

Any light source within the infrared region is applicable to exposure of the thermally developable photosensitive material and infrared semiconductor lasers (780 nm, 820 nm) are preferred in terms of high power and transmission capability through the photosensitive material.

In the invention, exposure is preferably conducted by laser scanning exposure. It is also preferred to use a laser exposure apparatus, in which scanning laser light is not exposed at an angle substantially vertical to the exposed surface of the photosensitive material. The expression "laser light is not exposed at an angle substantially vertical to the exposed surface" means that laser light is exposed preferably at an angle of 55 to 88°, more preferably 60 to 86°, still more preferably 65 to 84, and optimally 70 to 82°. When the photosensitive material is scanned with laser light, the beam spot diameter on the surface of the photosensitive material is preferably not more than 200  $\mu\text{m}$ , and more preferably not more than 100  $\mu\text{m}$ . Thus, the less spot diameter preferably reduces an angle displacing from verticality of the laser incident angle. The lower limit of the beam spot diameter is 10  $\mu\text{m}$ . The thus laser scanning exposure can reduce deterioration in image quality due to reflection light, such as occurrence of interference fringe-like unevenness.

Exposure applicable in the invention is conducted preferably using a laser scanning exposure apparatus producing longitudinally multiple scanning laser light, whereby deterioration in image quality such as occurrence of interference fringe-like unevenness is reduced, as compared to scanning laser light with longitudinally single mode. Longitudinal multiplication can be achieved by a technique of employing backing light with composing waves or a technique of high frequency overlapping. The expression "longitudinally multiple" means that the exposure wavelength is not a single wavelength. The exposure wavelength distribution is usually

not less than 5 nm and not more than 10 nm. The upper limit of the exposure wavelength distribution is not specifically limited but usually about 60 nm.

It is preferred that when subjected to thermal development, the photothermographic material contains an organic solvent. Examples of solvents include ketones such as acetone, isophorone, ethyl amyl ketone, methyl ethyl ketone, methyl isobutyl ketone; alcohols such as methyl alcohol, ethyl alcohol, n-propyl alcohol, isopropyl alcohol, n-butyl alcohol, isobutyl alcohol, diacetone alcohol, cyclohexanol, and benzyl alcohol; glycols such as ethylene glycol, dimethylene glycol, triethylene glycol, propylene glycol and hexylene glycol; ether alcohols such as ethylene glycol monomethyl ether, and dimethylene glycol monomethyl ether; ethers such as ethyl ether, dioxane, and isopropyl ether; esters such as ethyl acetate, butyl acetate, amyl acetate, and isopropyl acetate; hydrocarbons such as n-pentane, n-hexane, n-heptane, cyclohexene, benzene, toluene, xylene; chlorinated compounds such as chloromethyl, chloromethylene, chloroform, and dichlorobenzene; amines such as monomethylamine, dimethylamine, triethanol amine, ethylenediamine, and triethylamine; and water, formaldehyde, dimethylformaldehyde, nitromethane, pyridine, toluidine, tetrahydrofuran and acetic acid. The solvents are not to be construed as limiting these examples. These solvents may be used alone or in combination.

The solvent content in the photosensitive material can be adjusted by varying conditions such as temperature conditions at the drying stage after the coating stage. The solvent content can be determined by means of gas chromatography under the conditions suitable for detecting the solvent. The total solvent content (based on weight) of the photothermographic material used in the invention is preferably adjusted to be 5 to 1,000 mg per m<sup>2</sup> of the photothermographic material and more preferably 100 to 500 mg/m<sup>2</sup> (based on the weight of constituting components of the photosensitive material, except for a support). The solvent content within the range described above leads to a photothermographic material with low fog density as well as high sensitivity.

## EXAMPLES

The present invention will be further described based on examples but embodiments of the invention are by no means limited to these examples.

### Example 1

#### Preparation of a Subbed PET Photographic Support

Both surfaces of a biaxially stretched thermally fixed 175  $\mu\text{m}$  PET film, available on the market, was subjected to corona discharging at 8 w/m<sup>2</sup>·min. Onto one side of the film, the subbing coating composition a-1 described below was applied so as to form a dried layer thickness of 0.8  $\mu\text{m}$ , which was then dried. The resulting coating was designated Subbing Layer A-1. Onto the opposite surface, the subbing coating composition b-1 described below was applied to form a dried layer thickness of 0.8  $\mu\text{m}$ . The resulting coating was designated Subbing Layer B-1.

#### Subbing Coating Composition a-1

Latex solution (solid 30%) of  
a copolymer consisting of butyl acrylate  
(30 weight %), t-butyl acrylate (20 weight %)  
styrene (25 weight %) and 2-hydroxy  
ethyl acrylate (25 weight %)

-continued

|                                      |         |
|--------------------------------------|---------|
| (C-1)                                | 0.6 g   |
| Hexamethylene-1,6-bis (ethyleneurea) | 0.8 g   |
| Water to make                        | 1 liter |

#### Subbing Coating Composition b-1

|                                                                                                                                                                 |         |
|-----------------------------------------------------------------------------------------------------------------------------------------------------------------|---------|
| Latex liquid (solid portion of 30%)<br>of a copolymer consisting of<br>butyl acrylate (40 weight %)<br>styrene (20 weight %)<br>glycidyl acrylate (25 weight %) | 270 g   |
| (C-1)                                                                                                                                                           | 0.6 g   |
| Hexamethylene-1,6-bis(ethyleneurea)                                                                                                                             | 0.8 g   |
| Water to make                                                                                                                                                   | 1 liter |

Subsequently, the surfaces of Subbing Layers A-1 and B-1 were subjected to corona discharging with 8 w/m<sup>2</sup>·minute. Onto the Subbing Layer A-1, the upper subbing layer coating composition a-2 described below was applied so as to form a dried layer thickness of 0.8  $\mu\text{m}$ , which was designated Subbing Layer A-2, while onto the Subbing Layer B-1, the upper subbing layer coating composition b-2 was applied so as to form a dried layer thickness of 0.8  $\mu\text{m}$ , having a static preventing function, which was designated Subbing Upper Layer B-2.

#### Upper Subbing Layer Coating Composition a-2

|                                              |                      |
|----------------------------------------------|----------------------|
| Gelatin in an amount (weight) to make        | 0.4 g/m <sup>2</sup> |
| (C-1)                                        | 0.2 g                |
| (C-2)                                        | 0.2 g                |
| (C-3)                                        | 0.1 g                |
| Silica particles (av. size 3 $\mu\text{m}$ ) | 0.1 g                |
| Water to make                                | 1 liter              |

#### Upper Subbing Layer Coating Composition b-2

|                                       |         |
|---------------------------------------|---------|
| (C-4)                                 | 60 g    |
| Latex solution (solid 20% comprising) | 80 g    |
| (C-5) as a substituent                |         |
| Ammonium sulfate                      | 0.5 g   |
| (C-6)                                 | 12 g    |
| polyethylene glycol                   | 6 g     |
| (average molecular weight of 600)     |         |
| Water to make                         | 1 liter |

(C-1)



(C-2)



61

-continued



(C-3)



(C-4)

(Mn is a number average molecular weight)  
x:y = 75:25 (weight ratio)



(C-5)

p:g:r:s:t = 40:5:10:5:40 (weight ratio)



(C-6)

#### Preparation of Photosensitive Silver Halide Emulsion A

In 900 ml of deionized water were dissolved 7.5 g of gelatin and 10 mg of potassium bromide. After adjusting the temperature and the pH to 35° C. and 3.0, respectively, 370 ml of an aqueous solution containing 74 g silver nitrate and an equimolar aqueous solution containing potassium bromide, potassium iodide (in a molar ratio of 98 to 2) and  $1 \times 10^{-4}$  mol/mol Ag of iridium chloride were added over a period of 10 minutes by the controlled double-jet method,

62

while the pH was maintained at 7.7. Thereafter, 4-hydroxy-6-methyl-1,3,3a,7-tetraazaindene was added and the pH was adjusted to 5 using NaOH. There was obtained cubic silver iodobromide grains having an average grain size of 0.06  $\mu$ m, a variation coefficient of the projection area equivalent diameter of 12 percent, and the proportion of the {100} face of 87 percent. The resulting emulsion was flocculated to remove soluble salts, employing a flocculating agent and after desalting, 0.1 g of phenoxyethanol was added and the pH and pAg were adjusted to 5.9 and 7.5, respectively to obtain silver halide emulsion A.

#### Preparation of Powdery Organic Silver Salt A

In 4720 ml water were dissolved 111.4 g of behenic acid, 83.8 g of arachidic acid and 54.9 g of stearic acid at 80° C. The, after adding 540.2 ml of 1.5M aqueous sodium hydroxide solution with stirring and further adding 6.9 ml of concentrated nitric acid, the solution was cooled to a temperature of 55° C. to obtain an aqueous organic acid sodium salt solution. To the solution were added the silver halide emulsion obtained above (equivalent to 0.038 mol silver) and 450 ml water and stirring further continued for 5 min., while maintained at a temperature of 55° C. Subsequently, 760 ml of 1M aqueous silver nitrate solution was added in 2 min. and stirring continued further for 20 min., then, the reaction mixture was filtered to remove aqueous soluble salts. Thereafter, washing with deionized water and filtration were repeated until the filtrate reached a conductivity of 2  $\mu$ S/cm.

Using a flush jet dryer (produced by Seishin Kigyo Co., Ltd.), the thus obtained cake-like organic silver salt was dried under an atmosphere of inert gas (i.e., nitrogen gas) having a volume ratio shown in Table 1, according to the operation condition of a hot air temperature at the inlet of the dryer until reached a moisture content of 0.1%. The moisture content was measured by an infrared ray aquameter.

#### Preparation of Photosensitive Emulsion Dispersing Solution

In 1457 g methyl ethyl ketone was dissolved 14.57 g of polyvinyl butyral powder (Butvar B-79, available from Monsanto Corp.) and further thereto was gradually added 500 g of the powdery organic silver salt with stirring by a dissolver type homogenizer. Thereafter, the mixture was dispersed using a media type dispersion machine (available from Getzmann Corp.), which was packed 1 mm Zr beads (available from Toray Co. Ltd.) by 80%, at a circumferential speed of 13 m and for 3 min. of a retention time with a mill to obtain photosensitive emulsion dispersing solution to prepare photosensitive emulsion Nos. 101 through 113.

#### Preparation of Infrared Sensitizing Dye Solution

In 73.4 ml methanol were dissolved 350 mg of infrared sensitizing dye No. S-43, 13.96 g of 2-chlorobenzoic acid, and 2.14 g of 5-methyl-2-mercaptopbenzimidazole in a dark room to obtain an infrared sensitizing dye solution.

#### Preparation of Stabilizer Solution

Stabilizer 1 of 1.0 and potassium acetate of 0.5 g were dissolved in 8.5 g methanol to prepare a stabilizer solution.

#### Preparation of Developer Solution

Developer 1,1-bis(2-hydroxy-3,5-dimethylphenyl)-2-methylpropane of 17.74 g was dissolved in MEK to make 100 ml of a developer solution.

#### Preparation of Antifogging Solution

Antifogging 2 of 5.81 g was dissolved in MEK to make 100 ml of an antifogging solution.

#### Preparation of Photosensitive Layer Coating Composition

The photosensitive emulsion dispersing solution of 50 g and 15.11 g MEK were maintained at 21° C. with stirring. Then, antifogging 1 (390  $\mu$ l of 10% methanol solution) was added and stirred for 1 hr. and calcium bromide (996  $\mu$ l of

10% methanol solution) was added and further stirred for 30 min. Subsequently, 1.416 ml of an infrared sensitizing dye solution and 667  $\mu$ l stabilizer solution were added and stirred for 1 hr., then, the temperature was lowered to 13° C. and stirring was further conducted for 30 min. Next, 13.31 g of polyvinyl butyral (Butvar B-79, available from Monsanto Co.) was added thereto and stirred for 30 min., while being maintained at 13° C., thereafter, the following addenda were added at 15 min. intervals with stirring.

|                          |        |
|--------------------------|--------|
| Phthalazine              | 305 mg |
| Tetrachlorophthalic acid | 102 mg |
| 4-Methylphthalic acid    | 137 mg |
| Infrared dye 1           | 37 mg  |

After stirring the above composition for 15 min., the following addenda were successively added thereto with stirring to obtain a photosensitive layer coating solution.

|                                                     |          |
|-----------------------------------------------------|----------|
| Antifoggant solution                                | 5.47 ml  |
| Image stabilizer<br>[of formula (1) or (2)] Table 1 | 14.06 ml |
| Developer solution                                  |          |
| Crosslinking agent etc.<br>(as shown in Table 1)    | 1.60 ml  |
| 10% MEK solution                                    |          |

Drying was carried out at 75° C. for a period of 5 min.

#### Backing Layer coating

|   |                                                                                                   |                      |
|---|---------------------------------------------------------------------------------------------------|----------------------|
| 5 | Cellulose acetate<br>(10% methyl ethyl ketone solution)                                           | 15 ml/m <sup>2</sup> |
|   | Matting agent, monodisperse silica having<br>monodispersity of 15% and average size of 10 $\mu$ m | 30 mg/m <sup>2</sup> |

#### 10 Photosensitive Layer Coating

The coating solution thus prepared was coated so as to have a silver coverage of 2 g/m<sup>2</sup> and dried at 75° C. for a 15 period of 5 min. Drying was conducted in an atmosphere of nitrogen gas stream to inhibit adverse effects caused by oxygen.

#### 20 Surface Protective Layer

The following composition was coated on the photosensitive layer.

|    |                                                                                                  |                      |
|----|--------------------------------------------------------------------------------------------------|----------------------|
| 25 | Methyl ethyl ketone (MEK)                                                                        | 17 ml/m <sup>2</sup> |
|    | Cellulose acetate                                                                                | 2.3 g/m <sup>2</sup> |
|    | Matting agent, monodisperse silica having<br>monodispersity of 10% and average size of 4 $\mu$ m | 70 mg/m <sup>2</sup> |

Photothermographic material Samples 101 to 113 were prepared by incorporating an image stabilizer and cross-linking agent as shown in Table 1.



Infrared dye 1



Vinylsulfon compound



TABLE 1

| Sample | Drying Condition<br>N <sub>2</sub> /O <sub>2</sub> | Additive                |                            |                          | Remark |
|--------|----------------------------------------------------|-------------------------|----------------------------|--------------------------|--------|
|        |                                                    | Volume Ratio<br>(%)     | Crosslinking Agent<br>(mg) | Image Stabilizer<br>(mg) |        |
| 101    | 78/21                                              | None                    | None                       | Comp.                    |        |
| 102    | 85/15                                              | None                    | None                       | Inv.                     |        |
| 103    | 95/5                                               | None                    | None                       | Inv.                     |        |
| 104    | 78/21                                              | HDI + VSC<br>(200 + 50) | None                       | Comp.                    |        |
| 105    | 85/15                                              | HDI + VSC<br>(200 + 50) | None                       | Inv.                     |        |
| 106    | 95/5                                               | HDI + VSC<br>(200 + 50) | None                       | Inv.                     |        |
| 107    | 78/21                                              | HDI + VSC<br>(200 + 50) | BI-4<br>(2500)             | Comp.                    |        |
| 108    | 85/15                                              | HDI + VSC<br>(200 + 50) | BI-4<br>(2500)             | Inv.                     |        |
| 109    | 95/5                                               | HDI + VSC<br>(200 + 50) | BI-4<br>(2500)             | Inv.                     |        |
| 110    | 78/21                                              | HDI + VSC<br>(200 + 50) | I-1<br>(300)               | Comp.                    |        |
| 111    | 85/15                                              | HDI + VSC<br>(200 + 50) | I-1<br>(300)               | Inv.                     |        |
| 112    | 95/5                                               | HDI + VSC<br>(200 + 50) | I-1<br>(300)               | Inv.                     |        |
| 113    | 95/5                                               | HDI + VSC<br>(200 + 50) | I-1<br>(300)               | Inv.                     |        |

In the Table, HDI, HDSI and VSC represent hexamethylene diisocyanate, hexamethylene dithioisocyanate and vinylsulfon compounds, respectively.

#### Measurement of Solvent Content of Film

Film samples were each measured with respect to the solvent content. Thus, sample films each were cut to an area of 46.3 cm<sup>2</sup>, further finely cut to about 5 mm, contained into a specified Bayern bottle, which was closely packed with septum and aluminum cap, and set to head space sampler HP769 (available Hewlett Packard Co.), which was connected to gas chromatography (GC) Hewlett Packard type 5971 provided with a hydrogen flame ion detector (FID). Chromatograms were obtained under the measurement conditions including a head space sampler heating temperature of 120° C. for 20 min., a GC-introducing temperature of 150° C., column of DB-624 (available from J & W co.) and temperature-increasing of 45° C. (3 min.) to 100° C. at a rate of 8°/min. Solvents to be measure were methyl ethyl ketone and methanol. A given amount of each solvent, which was further diluted with butanol was contained into a Bayern bottle and subjected to the chromatographic measurement in a manner similar to above. Using a calibration curve prepared from the obtained chromatogram peak area, the solvent content of each film sample was determined.

Photothermographic material Samples 101 to 113 were aged under the condition A and measured according to the procedure described above. As a result, the solvent content thereof was within the range of 100 to 120 mg/m<sup>2</sup>.

#### Exposure and Development

Samples each were subjected to laser scanning exposure from the emulsion side using an exposure apparatus having a light source of 800 to 820 nm semiconductor laser of longitudinal multi-mode, which was made by means of high frequency overlapping. In this case, exposure was conducted at an angle between the exposed surface and exposing laser light was 75° and in an atmosphere at a temperature of 23° C. and 50% RH (and as a result, images with superior

sharpness were unexpectedly obtained, as compared to exposure at an angle of 90°). Using an automatic processor provided with a heated drum, subsequently, exposed samples were subjected to thermal development at 110° C. for 15 sec., while bringing the protective layer surface of the photosensitive material into contact with the drum surface. The thermal development was conducted in an atmosphere at 23° C. and 50% RH.

Thermally developed samples each were subjected to sensitometry using a densitometer and evaluated with respect to a fog density (i.e., minimum density and denoted as Dmin) and sensitivity. The sensitivity was represented by a relative value of reciprocal of exposure necessary to give a density of Dmin plus 1.0, based on the sensitivity of Sample 101 being 100.

#### Storage Stability

Samples each were allowed to stand for a period of 7 days under the condition A or B described below and subjected to exposure and development, as described above.

Condition A: 25° C. and 55% RH.

Condition b: 40° C. and 80% RH Images thus obtained were sensitometrically evaluated. The difference in the minimum density (also denoted as Dmin) between conditions A and B, i.e., Dmin(B)–Dmin(A) was determined as a measure of storage stability of unexposed photothermographic materials. Results thereof are shown in Table 2.

#### Image Lasting Quality

Samples were allowed to stand under the condition A for 7 days and then subjected to exposure and development in a manner similar to the above. Sample thus processed were further allowed to stand in an atmosphere at 25° C. and 55% RH under fluorescent lamps and after then, aged samples each were evaluated with respect to image tone, based on the following criteria:

- 5: No problem in image tone,
- 4: No problem in practical use in image tone,
- 3: Slightly yellowish but acceptable level,
- 2: Unfavored image tone and unacceptable level, and
- 1: Marked change observed and unacceptable level.

TABLE 2

| Sample | Aged under Condition A,<br>7 days |             | Storage | Image Lasting |         |
|--------|-----------------------------------|-------------|---------|---------------|---------|
|        | Fog                               | Sensitivity |         | Stability     | Quality |
| 101    | 0.54                              | 100         | 0.47    | 1             | Comp.   |
| 102    | 0.43                              | 103         | 0.40    | 1             | Inv.    |
| 103    | 0.39                              | 107         | 0.37    | 1             | Inv.    |
| 104    | 0.46                              | 103         | 0.42    | 1             | Comp.   |
| 105    | 0.40                              | 106         | 0.38    | 1             | Inv.    |
| 106    | 0.35                              | 109         | 0.35    | 1             | Inv.    |
| 107    | 0.23                              | 112         | 0.24    | 2             | Comp.   |
| 108    | 0.14                              | 115         | 0.14    | 4             | Inv.    |
| 109    | 0.09                              | 122         | 0.10    | 5             | Inv.    |
| 110    | 0.26                              | 110         | 0.25    | 2             | Comp.   |
| 111    | 0.13                              | 117         | 0.13    | 4             | Inv.    |
| 112    | 0.10                              | 120         | 0.11    | 5             | Inv.    |
| 113    | 0.11                              | 119         | 0.10    | 5             | Inv.    |

As is apparent from Table 2, the inventive samples, which were prepared under a gas atmosphere containing increased inert gas fraction, exhibited low fogging and superior raw stock stability, compared to the comparative samples. Specifically, samples containing a cross-linking agent and an image stabilizer exhibited superior raw stock stability and image lasting quality as well as enhanced sensitivity.

**67**  
Example 2

On a photosensitive layer side of a commercially available, biaxially stretched, thermally fixed and blue-tinted 75  $\mu\text{m}$  PET film, subbing layers A-1 and A-2 were nd subbing layers B-1 and B-2 were coated on the opposite side of the support in a manner similar to Example 1 to prepare a photographic support.

Photosensitive silver halide emulsion A and powdery organic silver salt A were prepared similarly to example 1 to prepare a photosensitive emulsion dispersing solution. Using these, photothermographic material Samples 201 to 213 were prepared similarly to Example 1, except that, an image stabilizer and a cross-linking agent of an epoxy compound represented by formula (9) or an acid anhydride were used as shown in Table 3.

TABLE 3

| Sample | Drying Condition<br>$\text{N}_2/\text{O}_2$ | Additive               |                         |                       | Remark |
|--------|---------------------------------------------|------------------------|-------------------------|-----------------------|--------|
|        |                                             | Volume Ratio (%)       | Crosslinking Agent (mg) | Image Stabilizer (mg) |        |
| 201    | 78/21                                       | EP-1 + B-11 (200 + 50) | None                    | Comp.                 |        |
| 202    | 85/15                                       | EP-1 + B-11 (200 + 50) | None                    | Inv.                  |        |
| 203    | 95/5                                        | EP-1 + B-11 (200 + 50) | None                    | Inv.                  |        |
| 204    | 78/21                                       | EP-1 + B-11 (200 + 50) | BI-4 (2500)             | Comp.                 |        |
| 205    | 85/15                                       | EP-1 + B-11 (200 + 50) | BI-4 (2500)             | Inv.                  |        |
| 206    | 95/5                                        | EP-1 + B-11 (200 + 50) | BI-4 (2500)             | Inv.                  |        |
| 207    | 78/21                                       | EP-1 + B-11 (200 + 50) | I-33 (300)              | Comp.                 |        |
| 208    | 85/15                                       | EP-1 + B-11 (200 + 50) | I-33 (300)              | Inv.                  |        |
| 209    | 95/5                                        | EP-1 + B-11 (200 + 50) | I-33 (300)              | Inv.                  |        |
| 210    | 95/5                                        | EP-9 + B-11 (200 + 50) | BI-4 (2500)             | Inv.                  |        |
| 211    | 95/5                                        | EP-9 + B-11 (200 + 50) | BI-3 (300)              | Inv.                  |        |
| 212    | 95/5                                        | EP-9 + B-11 (200 + 50) | I-1 (300)               | Inv.                  |        |
| 213    | 95/5                                        | EP-9 + B-11 (200 + 50) | I-33 (300)              | Inv.                  |        |

Storage stability of unexposed photothermographic al samples and image stability of processed samples valuated similarly to Example 4. Results thereof are shown in Table 4. Sensitivity is represented by a relative ased on the sensitivity of Sample 201 aged under the condition A being 100.

TABLE 4

| Sample | Aged under Condition A, 7 days |             | Storage | Image Lasting |         |
|--------|--------------------------------|-------------|---------|---------------|---------|
|        | Fog                            | Sensitivity |         | Stability     | Quality |
| 201    | 0.48                           | 100         | 0.49    | 1             | Comp.   |
| 202    | 0.43                           | 101         | 0.42    | 1             | Comp.   |
| 203    | 0.39                           | 105         | 0.38    | 1             | Inv.    |
| 204    | 0.24                           | 109         | 0.26    | 2             | Comp.   |
| 205    | 0.16                           | 112         | 0.18    | 4             | Inv.    |
| 206    | 0.12                           | 119         | 0.12    | 5             | Inv.    |

TABLE 4-continued

| 5  | Aged under Condition A, 7 days |       | Storage     | Image Lasting |         |        |
|----|--------------------------------|-------|-------------|---------------|---------|--------|
|    | Sample                         | Fog   | Sensitivity | Stability     | Quality | Remark |
| 10 | 207                            | 0.25  | 108         | 0.25          | 2       | Comp.  |
|    | 208                            | 0.15  | 113         | 0.16          | 4       | Inv.   |
|    | 209                            | 0.10  | 120         | 0.11          | 5       | Inv.   |
|    | 210                            | 0.11  | 120         | 0.12          | 5       | Inv.   |
|    | 211                            | 10.11 | 117         | 0.13          | 5       | Inv.   |
|    | 212                            | 10.10 | 119         | 0.12          | 5       | Comp.  |
|    | 213                            | 10.12 | 119         | 0.12          | 5       | Inv.   |

As is apparent from Table 4, the inventive samples, which were prepared under a gas atmosphere containing increased inert gas fraction, exhibited low fogging and superior raw stock stability, compared to the comparative samples. Specifically, samples containing a cross-linking agent and an image stabilizer exhibited superior raw stock stability and image lasting quality as well as enhanced sensitivity.

Example 3

25 On a photosensitive layer side of a commercially available, biaxially stretched, thermally fixed and blue-tinted 175  $\mu\text{m}$  PET film, subbing layers A-1 and A-2 were coated and subbing layers B-1 and B-2 were coated on the opposite side of the support in a manner similar to Example 1 to prepare a photographic support.

Photosensitive silver halide emulsion A and powdery organic silver salt A were prepared similarly to example 1 to prepare a photosensitive emulsion dispersing solution. Using these, photothermographic material Samples 301 to 35 308 were prepared similarly to Example 1, in which supersensitizer 5-methyl-2-mercaptopbenzimidazole (M-4) was contained or not, and image stabilizer and a crosslinking agent were used as shown in Table 5.

TABLE 5

| 45 | Drying Condition | Additive                                 |                                   |                       | Remark |
|----|------------------|------------------------------------------|-----------------------------------|-----------------------|--------|
|    |                  | $\text{N}_2/\text{O}_2$ Volume Ratio (%) | Crosslinking Agent (mg)           | Image Stabilizer (mg) |        |
| 50 | 301              | 85/15                                    | HDI + VSC (200 + 50)              | BI-3 (2500)           | Inv.   |
|    | 302              | 95/5                                     | HDI + VSC (200 + 50)              | BI-3 (2500)           | Inv.   |
|    | 303              | 85/15                                    | HDI + VSC + M-4 (200 + 50 + 45)   | BI-3 (2500)           | Inv.   |
|    | 304              | 95/5                                     | HDI + VSC + M-4 (200 + 50 + 45)   | BI-3 (2500)           | Inv.   |
|    | 305              | 85/15                                    | EP-9 + B-11 (200 + 50)            | I-4 (300)             | Inv.   |
|    | 306              | 95/5                                     | EP-9 + B-11 (200 + 50)            | I-4 (300)             | Inv.   |
|    | 307              | 85/15                                    | EP-9 + B-11 + M-4 (200 + 50 + 45) | I-4 (300)             | Inv.   |
|    | 308              | 95/5                                     | EP-9 + B-11 + M-4 (200 + 50 + 45) | I-4 (300)             | Inv.   |

55 In the Table, HDI, HDSI and VSC represent hexamethylene diisocyanate, hexamethylene dithioisocyanate and vinylsulfon compounds, respectively.

60 Storage stability of unexposed photothermographic material samples and image stability of processed samples were evaluated similarly to Example 1, provided that Sample

were aged for a period of 9 days. Results thereof are shown in Table 6. Sensitivity is represented by a relative value, based on the sensitivity of Sample 301 or 308 aged under the condition A being 100.

TABLE 6

| Sample | Aged under<br>Condition A,<br>9 days |             | Storage | Image<br>Lasting |         |
|--------|--------------------------------------|-------------|---------|------------------|---------|
|        | Fog                                  | Sensitivity |         | Stability        | Quality |
| 301    | 0.35                                 | 27          | 0.39    | 1                | Inv.    |
| 302    | 0.23                                 | 35          | 0.28    | 2                | Inv.    |
| 303    | 0.25                                 | 100         | 0.27    | 2                | Inv.    |
| 304    | 0.11                                 | 110         | 0.13    | 5                | Inv.    |
| 305    | 0.32                                 | 29          | 0.35    | 1                | Inv.    |
| 306    | 0.22                                 | 38          | 0.24    | 2                | Inv.    |
| 307    | 0.24                                 | 100         | 0.25    | 2                | Inv.    |
| 308    | 0.10                                 | 115         | 0.13    | 5                | Inv.    |

As apparent from Table 6, the inventive samples, which were prepared under a gas atmosphere containing increased inert gas fraction, exhibited low fogging and superior raw stock ability, compared to the comparative samples. Specifically, samples containing supersensitizer M-4 exhibited superior raw stock stability and image lasting quality as well as enhanced sensitivity.

#### Example 4

Photothermographic material samples No. 401 through 413 were prepared in the same manner as photothermographic material samples No. 101 through 113. Each of the samples was put in a barrier bag in a gas atmosphere having a composition as shown in Table 7.

TABLE 7

| Sample | Storage<br>Condition | Additive                                              |                               |                             | Remark |
|--------|----------------------|-------------------------------------------------------|-------------------------------|-----------------------------|--------|
|        |                      | N <sub>2</sub> /O <sub>2</sub><br>Volume<br>Ratio (%) | Crosslinking<br>Agent<br>(mg) | Image<br>Stabilizer<br>(mg) |        |
| 401    | 78/21                | None                                                  | None                          | Comp.                       |        |
| 402    | 85/15                | None                                                  | None                          | Inv.                        |        |
| 403    | 95/5                 | None                                                  | None                          | Inv.                        |        |
| 404    | 78/21                | HDI + VSC<br>(200 + 50)                               | None                          | Comp.                       |        |
| 405    | 85/15                | HDI + VSC<br>(200 + 50)                               | None                          | Inv.                        |        |
| 406    | 95/5                 | HDI + VSC<br>(200 + 50)                               | None                          | Inv.                        |        |
| 407    | 78/21                | HDI + VSC<br>(200 + 50)                               | BI-4<br>(2500)                | Comp.                       |        |
| 408    | 85/15                | HDI + VSC<br>(200 + 50)                               | BI-4<br>(2500)                | Inv.                        |        |
| 409    | 95/5                 | HDI + VSC<br>(200 + 50)                               | BI-4<br>(2500)                | Inv.                        |        |
| 410    | 78/21                | HDI + VSC<br>(200 + 50)                               | I-1<br>(300)                  | Comp.                       |        |
| 411    | 85/15                | HDI + VSC<br>(200 + 50)                               | I-1<br>(300)                  | Inv.                        |        |
| 412    | 95/5                 | HDI + VSC<br>(200 + 50)                               | I-1<br>(300)                  | Inv.                        |        |
| 413    | 95/5                 | HDSI + VSC<br>(200 + 50)                              | I-1<br>(300)                  | Inv.                        |        |

#### Measurement of Solvent Content of Film

Film samples were each measured with respect to the solvent content in a manner similar to Example 1. Thus, samples No. 401 to 413 were aged under the following

condition A and measured according to the procedure described above. As a result, the solvent content thereof was within the range of 100 to 120 mg/m<sup>2</sup>.

#### Exposure and Development

Samples each were subjected to exposure and thermal development and evaluated similarly to Example 1. The sensitivity was represented by a relative value of reciprocal of exposure necessary to give a density of Dmin plus 1.0, based on the sensitivity of Sample 401 being 100.

#### Storage Stability

Samples each were allowed to stand for a period of 10 days under the condition A or B described below and subjected to exposure and development, as described above.

Condition A: 25° C. and 55% RH.

Condition b: 40° C. and 80% RH

Images thus obtained were sensitometrically evaluated. The difference in the minimum density (also denoted as Dmin) between conditions A and B, i.e., Dmin(B)–Dmin(A) was determined as a measure of storage stability of unexposed photothermographic materials. Results thereof are shown in Table 8.

#### Image Lasting Quality

Samples were allowed to stand under the Condition A for 10 days and then subjected to exposure and development in a manner similar to the above. Sample thus processed were further allowed to stand in an atmosphere at 25° C. and 55% RH under fluorescent lamps and after then, aged samples each were evaluated with respect to image tone, based on the following criteria:

5: No problem in image tone,

4: No problem in practical use in image tone,

3: Slightly yellowish but acceptable level,

2: Unfavored image tone and unacceptable level, and

1: Marked change observed and unacceptable level.

TABLE 8

| Sample | Aged under<br>Condition A,<br>10 days |             | Storage | Image<br>Lasting |         |
|--------|---------------------------------------|-------------|---------|------------------|---------|
|        | Fog                                   | Sensitivity |         | Stability        | Quality |
| 401    | 0.44                                  | 100         | 0.38    | 1                | Comp.   |
| 402    | 0.33                                  | 105         | 0.30    | 1                | Inv.    |
| 403    | 0.29                                  | 109         | 0.29    | 2                | Inv.    |
| 404    | 0.40                                  | 102         | 0.42    | 1                | Comp.   |
| 405    | 0.31                                  | 110         | 0.28    | 2                | Inv.    |
| 406    | 0.25                                  | 120         | 0.26    | 2                | Inv.    |
| 407    | 0.15                                  | 118         | 0.18    | 3                | Comp.   |
| 408    | 0.10                                  | 120         | 0.11    | 5                | Inv.    |
| 409    | 0.06                                  | 125         | 0.08    | 5                | Inv.    |
| 410    | 0.16                                  | 117         | 0.18    | 3                | Comp.   |
| 411    | 0.11                                  | 122         | 0.12    | 5                | Inv.    |
| 412    | 0.07                                  | 124         | 0.09    | 5                | Inv.    |
| 413    | 0.08                                  | 126         | 0.09    | 5                | Inv.    |

As is apparent from Table 8, the inventive samples exhibited low fogging and superior raw stock stability, compared to the comparative samples. Specifically, samples containing a cross-linking agent and an image stabilizer exhibited superior raw stock stability and image lasting quality as well as enhanced sensitivity.

It was further confirmed that in cases when the compound capable of generation a labile halogen atom upon exposure to ultraviolet or visible light was not used in combination, image lasting quality was slightly deteriorated.

Photographic material samples No. 501 through 513 were prepared in the same manner as samples No. 201 through 213 in Example 2.

TABLE 9

| Sample | Storage Condition N <sub>2</sub> /O <sub>2</sub> | Additive               |                         |                       | Remark |
|--------|--------------------------------------------------|------------------------|-------------------------|-----------------------|--------|
|        |                                                  | Volume Ratio (%)       | Crosslinking Agent (mg) | Image Stabilizer (mg) |        |
| 501    | 78/21                                            | EP-1 + B-11 (200 + 50) | None                    | Comp.                 |        |
| 502    | 85/15                                            | EP-1 + B-11 (200 + 50) | None                    | Inv.                  |        |
| 503    | 95/5                                             | EP-1 + B-11 (200 + 50) | None                    | Inv.                  |        |
| 504    | 78/21                                            | EP-1 + B-11 (200 + 50) | BI-4 (2500)             | Comp.                 |        |
| 505    | 85/15                                            | EP-1 + B-11 (200 + 50) | BI-4 (2500)             | Inv.                  |        |
| 506    | 95/5                                             | EP-1 + B-11 (200 + 50) | BI-4 (2500)             | Inv.                  |        |
| 507    | 78/21                                            | EP-1 + B-11 (200 + 50) | I-33 (300)              | Comp.                 |        |
| 508    | 85/15                                            | EP-1 + B-11 (200 + 50) | I-33 (300)              | Inv.                  |        |
| 509    | 95/5                                             | EP-1 + B-11 (200 + 50) | I-33 (300)              | Inv.                  |        |
| 510    | 95/5                                             | EP-9 + B-11 (200 + 50) | BI-4 (2500)             | Inv.                  |        |
| 511    | 95/5                                             | EP-9 + B-11 (200 + 50) | BI-3 (300)              | Inv.                  |        |
| 512    | 95/5                                             | EP-9 + B-11 (200 + 50) | I-1 (300)               | Inv.                  |        |
| 513    | 95/5                                             | EP-9 + B-11 (200 + 50) | I-33 (300)              | Inv.                  |        |

Storage stability of unexposed photothermographic material samples and image stability of processed samples were evaluated similarly to Example 4. Results thereof are shown in Table 10. Sensitivity is represented by a relative value, based on the sensitivity of Sample 501 aged under the condition A being 100.

TABLE 10

| Sample | Aged under Condition A, 7 days |             | Storage | Image Lasting |         |
|--------|--------------------------------|-------------|---------|---------------|---------|
|        | Fog                            | Sensitivity |         | Stability     | Quality |
| 501    | 0.46                           | 100         | 0.45    | 1             | Comp.   |
| 502    | 0.35                           | 104         | 0.32    | 1             | Inv.    |
| 503    | 0.30                           | 106         | 0.31    | 2             | Inv.    |
| 504    | 0.16                           | 113         | 0.19    | 3             | Comp.   |
| 505    | 0.11                           | 119         | 0.12    | 5             | Inv.    |
| 506    | 0.08                           | 125         | 0.11    | 5             | Inv.    |
| 507    | 0.15                           | 112         | 0.16    | 3             | Comp.   |
| 508    | 0.12                           | 123         | 0.10    | 5             | Inv.    |
| 509    | 0.09                           | 125         | 0.09    | 5             | Inv.    |
| 510    | 0.09                           | 126         | 0.10    | 5             | Inv.    |
| 511    | 0.08                           | 127         | 0.09    | 5             | Inv.    |
| 512    | 0.07                           | 129         | 0.08    | 5             | Inv.    |
| 513    | 0.08                           | 128         | 0.09    | 5             | Inv.    |

As is apparent from Table 10, the inventive samples exhibited low fogging and superior raw stock stability, compared to the comparative samples. Specifically, samples containing a cross-linking agent and an image stabilizer exhibit superior raw stock stability and image lasting quality as well as enhanced sensitivity.

Effects of a deoxidant were evaluated according to the following procedure.

Preparation of Deoxidant Package

5 Powdery iron having a mean granularity of 60 mesh of 20 g was put in a package formed of polypropylene unwoven fabric FSP1050 (produced by Asahi Chemicals Co., Ltd.) exhibiting METSUE of 70 g/m<sup>2</sup> and a Garley gas-permeability of 4 sec/100 ml and sealed using Fuji Impulse Sealer FI-K400-5 (produced by Fuji Seisakusho and commercially available from Mitsubishi Co. Ltd.) to obtain a deoxidant package.

Package containing Deoxidant Package

10 15 Photothermographic material samples 408 and 411 of example 4 were each cut to a sheets of 25.4×30.5 cm and were held sheet by sheet with thin paper interleaf to obtain a sample package having 100 sheets as a package unit. The thus obtained sample package and the deoxidant package were put into a light-shielding moisture-resistant bag and sealed under an inert gas atmosphere (N<sub>2</sub>/O<sub>2</sub>=85/15 by volume). Further, a comparative package containing no deoxidant was also prepared. The sealed packages were aged at room temperature, and after 500 days, the packages were opened and photothermographic samples were evaluated similarly to Example 4. Results are shown in Table 11. Sensitivity was represented by a relative value, based on the sensitivity of the sample containing no deoxidant being 100.

TABLE 11

| Sample | Deoxidant | Raw Stock Stability |      | Image Lasting |         |
|--------|-----------|---------------------|------|---------------|---------|
|        |           | Sensitivity         | Fog  | Quality       | Remarks |
| 408    | No        | 100                 | 0.18 | 4             | Comp.   |
| 408    | Yes       | 105                 | 0.13 | 5             | Inv.    |
| 411    | No        | 100                 | 0.19 | 4             | Inv.    |
| 411    | Yes       | 104                 | 0.14 | 5             | Inv.    |

40 45 Samples which were aged in the presence of the deoxidant exhibited low fogging as well as high sensitivity and superior image fastness.

What is claimed is:

1. A method for preparing a photothermographic material comprising an organic silver salt, wherein the method comprises the steps of:

(a) preparing an emulsion containing an organic silver salt and a silver halide,

(b) drying the emulsion,

(c) coating the emulsion, and

(d) drying the coated emulsion,

and wherein at least one of the steps (a) through (d) is conducted under the gas atmosphere containing an inert gas having a volume fraction of not less than 85% or under a gas atmosphere containing oxygen gas having a volume fraction of not more than 15%.

50 55 2. The method of claim 1, wherein step (b) is conducted under the gas atmosphere containing an inert gas having a volume fraction of not less than 85% or under a gas atmosphere containing oxygen gas having a volume fraction of not more than 15%.

60 65 3. The method of claim 2, wherein step (b), the emulsion is dried at a temperature of 35 to 80° C.

4. The method of claim 1, wherein the inert gas is at least one selected from the group consisting of nitrogen, helium and argon.

5. The method of claim 1, wherein the photothermographic material further comprises a light sensitive silver halide, a reducing agent and a binder.

6. The method of claim 5, wherein the photothermographic material further comprises a cross-linking agent.

7. The method of claim 6, wherein the photothermographic material further comprises a compound capable of generating a labile species other than a halogen atom upon exposure to ultraviolet ray or visible light to deactivate the reducing agent.

8. The method of claim 7, wherein the labile species other than a halogen atom is a free radical comprised of plural atoms.

9. The method of claim 6, wherein the cross-linking agent is selected from the group consisting of an epoxy compound, acid anhydride, an isocyanate compound, and an isothiocyanate compound.

10. A method of preparing a package containing a photothermographic material comprising an organic silver salt, wherein the method comprises the steps of:

- (a) preparing an emulsion containing an organic silver salt and a silver halide,
- (b) drying the emulsion,
- (c) coating the emulsion,
- (d) drying the coated emulsion to prepare a photothermographic material, and
- (e) packaging the photothermographic material to prepare a package containing the photothermographic material and wherein at least one of the steps (a) through (e) is conducted under the gas atmosphere containing an inert gas having a volume fraction of not less than 85% or

under a gas atmosphere containing oxygen gas having a volume fraction of not more than 15%.

11. The method of claim 10, wherein step (e) is conducted under the gas atmosphere containing an inert gas having a volume fraction of not less than 85% or under a gas atmosphere containing oxygen gas having a volume fraction of not more than 15%.

12. The method of claim 10, wherein the inert gas is at least one selected from the group consisting of nitrogen, helium and argon.

13. The method of claim 10, wherein the photothermographic material further comprises a light sensitive silver halide, a reducing agent and a binder.

14. A package containing a photothermographic material, wherein the package is filled with a gas containing an inert gas having a volume fraction of not less than 85% or with a gas containing oxygen gas having a volume fraction of not more than 15%.

15. The package of claim 14, wherein the inert gas is at least one selected from the group consisting of nitrogen, helium, and argon.

16. The package of claim 14, wherein the package further contains a deoxidant.

17. The package of claim 16, wherein the deoxidant is at least one selected from the group consisting of ferrous salts, iron powder, sulfites, hydrogen sulfites, dithionites, hydroquinone, catechol, resorcinol, pyrogallol, gallic acid, Rongalit, ascorbic acid, ascorbates, isoascorbic acid, isoascorbates, sorbose, glycose, lignin, dibutylhydroxytoluene and butylhydroxyanisole.

\* \* \* \* \*